



US006514662B2

(12) **United States Patent**  
**Ito**

(10) **Patent No.:** **US 6,514,662 B2**  
(b4) **Date of Patent:** **Feb. 4, 2003**

(54) **PHOTOTHERMOGRAPHIC MATERIAL**(75) Inventor: **Tadashi Ito, Minami-ashigara (JP)**(73) Assignee: **Fuji Photo Film Co., Ltd., Kanagawa (JP)**

(\*) Notice: Subject to any disclaimer, the term of this patent is extended or adjusted under 35 U.S.C. 154(b) by 0 days.

(21) Appl. No.: **09/799,076**(22) Filed: **Mar. 6, 2001**(65) **Prior Publication Data**

US 2001/0044069 A1 Nov. 22, 2001

(30) **Foreign Application Priority Data**

Mar. 6, 2000 (JP) ..... 2000-060122

(51) **Int. Cl.<sup>7</sup>** ..... **G03C 1/498; G03C 1/76; G03C 5/29**(52) **U.S. Cl.** ..... **430/264; 430/353; 430/496; 430/523; 430/536; 430/619; 430/961**(58) **Field of Search** ..... 430/619, 264, 430/353, 961, 536, 496, 523(56) **References Cited**

## U.S. PATENT DOCUMENTS

3,841,872 A 10/1974 Burness et al. ..... 430/622

|                |         |                      |         |
|----------------|---------|----------------------|---------|
| 5,545,507 A    | 8/1996  | Simpson et al. ....  | 430/619 |
| 5,561,038 A    | 10/1996 | Goan .....           | 430/567 |
| 6,027,871 A    | 2/2000  | Katoh .....          | 430/619 |
| 6,268,118 B1 * | 7/2001  | Iwasaki et al. ....  | 430/620 |
| 6,274,302 B1 * | 8/2001  | Watanabe et al. .... | 430/619 |
| 6,277,554 B1 * | 8/2001  | Kamada et al. ....   | 430/619 |
| 6,309,814 B1 * | 10/2001 | Ito .....            | 430/619 |

\* cited by examiner

*Primary Examiner*—Richard L. Schilling(74) *Attorney, Agent, or Firm*—Birch, Stewart, Kolasch & Birch, LLP(57) **ABSTRACT**

A photothermographic material having an image-forming layer that contains at least a non-photosensitive silver salt of an organic acid, a photosensitive silver halide, a nucleating agent and a binder on a support, and a protective layer at a position remoter from the support compared with the image-forming layer, which shows a saturation swelling time of 60 seconds or longer in distilled water at 21° C. According to the present invention, there is provided a photothermographic material for photographic art, in particular, for scanners, image setters and so forth, which shows low humidity dependency during development for developed character line width and can secure high image density (Dmax) even in a low humidity environment.

**25 Claims, 1 Drawing Sheet**

Fig. 1



## PHOTOTHERMOGRAPHIC MATERIAL

## FIELD OF THE INVENTION

The present invention relates to a photothermographic material. In particular, the present invention relates to a photothermographic material for scanners, image setters and so forth, which is particularly suitable for photographic art. More precisely, the present invention relates to a photothermographic material that shows low humidity dependency during development for developed character line width and can secure high image density (Dmax) even in a low humidity environment.

## BACKGROUND OF THE INVENTION

There are known many photosensitive materials having a photosensitive layer on a support, with which image formation is attained by imagewise light exposure. Those materials include those utilizing a technique of forming images by heat treatment as systems that can contribute to the environmental protection and simplify image-forming means.

In recent years, reduction of amount of waste processing solutions is strongly desired in the field of photographic art from the standpoints of environmental protection and space savings. Therefore, development of techniques relating to photothermographic materials for photographic art is required, which materials enable efficient exposure by a laser scanner or laser image setter and formation of clear black images having high resolution and sharpness. Such photothermographic materials can provide users with simpler and non-polluting heat development processing systems that eliminate the use of solution-type processing chemicals.

Methods for forming images by heat development are described in, for example, U.S. Pat. Nos. 3,152,904 and 3,457,075 and D. Klosterboer, "Thermally Processed Silver Systems A", Imaging Processes and Materials, Neblette, 8th ed., compiled by J. Sturge, V. Walworth and A. Shepp, Chapter 9, p.279, (1989). Such photothermographic materials comprise a reducible non-photosensitive silver salt (e.g., silver salt of an organic acid), a photocatalyst (e.g., silver halide) in a catalytically active amount and a reducing agent for silver, which are usually dispersed in an organic binder matrix. While the photosensitive materials are stable at an ordinary temperature, when they are heated to a high temperature (e.g., 80° C. or higher) after light exposure, silver is produced through an oxidation-reduction reaction between the reducible silver salt (which functions as an oxidizing agent) and the reducing agent. The oxidation-reduction reaction is accelerated by catalytic action of a latent image generated upon exposure. The silver produced from the reaction of the reducible silver salt in the exposed areas shows black color and provides contrast with respect to the non-exposed areas, and thus images are formed.

In many of conventionally known photothermographic materials, an image-forming layer is formed by coating a coating solution using an organic solvent such as toluene, methyl ethyl ketone (MEK) and methanol as a solvent. However, not only use of an organic solvent as a solvent adversely affect human bodies during the production process, but also it is disadvantageous in view of cost because it requires process steps for recovery of the solvent and so forth.

Accordingly, methods of forming an image-forming layer by coating a coating solution using water as a solvent have been proposed. For example, Japanese Patent Laid-open

Publication (Kokai, hereinafter referred to as JP-A) 49-52626, JP-A-53-116144 and so forth disclose image-forming layers utilizing gelatin as a binder, and JP-A-50-151138 discloses an image-forming layer utilizing polyvinyl alcohol as a binder. Furthermore, JP-A-60-61747 discloses an image-forming layer utilizing gelatin and polyvinyl alcohol in combination. As another example, JP-A-58-28737 discloses an image-forming layer utilizing a water-soluble polyvinyl acetal as a binder. If these binders are used, 5 image-forming layers can be formed by using a coating solution comprising an aqueous solvent, and therefore considerable merits can be obtained with respect to environment and cost.

However, when a polymer such as gelatin, polyvinyl alcohol or water-soluble polyacetal is used as a binder, silver tone of developed areas becomes brown or yellow, which quite differs from black color regarded as a preferred proper color, and in addition, there arises, for example, a problem that the blacking density in exposed areas is low and the 10 density in unexposed areas is high. Thus, there can be obtained only images of which commercial value is seriously impaired. Furthermore, since such polymers show bad compatibility with the silver salt of an organic acid, there may also arise a problem that practically acceptable coatings 15 cannot be obtained in view of coated surface quality.

European Patent Publication (hereinafter referred to as EP-A) 762,196, JP-A-9-90550 and so forth disclose that high-contrast photographic property can be obtained by incorporating Group VII or VIII metal ions or metal complex ions into photosensitive silver halide grains for use in photothermographic materials, or incorporating a hydrazine derivative into the photosensitive materials.

For use of photographic art films in the fields of newspaper printing, commercial printing and so forth, there have 35 generally been desired systems that can provide stable images at any time. However, photothermographic materials showing such high-contrast photographic property as mentioned above, which is required for photographic art films, suffer from a problem that they show higher humidity dependency of character line width during development 40 compared with conventional films to be treated with chemicals.

Therefore, it has been desired to provide a photothermographic material that shows low humidity dependency of character line width during development and thus is suitable 45 for use in photographic art.

## SUMMARY OF THE INVENTION

50 Therefore, a first object to be achieved by the present invention is to provide a photothermographic material that shows low humidity dependency of character line width during development and can secure high image density (Dmax) even in a low humidity environment, in particular, as a photothermographic material for photographic art, more specifically, a photothermographic material for scanners, image setters and so forth.

55 A second object to be achieved by the present invention is to provide a photothermographic material that can be prepared by coating of an aqueous system, which is advantageous for the aspects of environment and cost.

The inventors of the present invention assiduously studied in order to achieve the aforementioned objects. As a result, they found that an excellent photothermographic material that provides the desired effects could be obtained by preparing a photothermographic material so that the material could have a saturation swelling time of 60 seconds or 60

longer in distilled water at 21° C., and thus accomplished the present invention.

That is, the present invention provides a photothermographic material having an image-forming layer that contains at least a non-photosensitive silver salt of an organic acid, a photosensitive silver halide, a nucleating agent and a binder on a support, and a protective layer at a position remoter from the support compared with the image-forming layer, which shows a saturation swelling time of 60 seconds or longer in distilled water at 21° C.

Preferably, the saturation swelling time is 80 seconds or longer.

Preferably, the binder of the image-forming layer comprises 50 weight % or more of latex of a polymer showing a glass transition temperature of -30° C. to 40° C.

Preferably, the protective layer has a thickness of 3  $\mu\text{m}$  or more.

According to another aspect of the present invention, there is provided a method for forming images, which comprises subjecting the aforementioned photothermographic material of the present invention to a heat treatment at a line speed of 140 cm/minute or higher.

According to a further aspect of the present invention, there is provided a method for forming images, which comprises exposing the aforementioned photothermographic material of the present invention for an exposure time of  $10^{-7}$  second or less.

According to a still further aspect of the present invention, there is provided a method for forming images, which comprises exposing the aforementioned photothermographic material of the present invention by using a multi-channel light source having two or more of laser heads.

According to the present invention, there can be obtained photographic properties suitable for photographic art including low development humidity dependency for line width and feasibility of securing sufficient image density (D<sub>max</sub>) even in a low humidity environment. Further, it enables coating with an aqueous system, which is advantageous for environment and cost.

#### BRIEF DESCRIPTION OF THE DRAWING

FIG. 1 is a side view of an exemplary heat developing apparatus used for heat development of the photothermographic material of the present invention. In the figure, there are shown a photothermographic material 10, carrying-in roller pairs 11, carrying-out roller pairs 12, rollers 13, a flat surface 14, heaters 15, and guide panels 16. The apparatus consists of a preheating section A, a heat development section B, and a gradual cooling section C.

#### PREFERRED EMBODIMENT OF THE INVENTION

The present invention will be explained in detail hereafter with respect to its embodiments and methods for practicing it. In the present specification, ranges indicated with “-” mean ranges including the numerical values before and after “-” as the minimum and maximum values.

In the photothermographic material of the present invention, humidity dependency of character line width during development can be lowered and high image density (D<sub>max</sub>) can be secured even in a low humidity environment, because the material is prepared to have a saturation swelling time of 60 seconds or longer in distilled water at 21° C.

As a main binder of the layers on the image-forming layer side, polymer latex that provides good photographic properties and enables coating with an aqueous system is preferably used.

The saturation swelling time in distilled water at 21° C. of the photothermographic material of the present invention is 60 seconds or longer, preferably 80 seconds or longer. Although the upper limit of the saturation swelling time is not particularly limited, it is preferably 5 minutes or shorter for practical use. Generally, the saturation swelling time can be measured by using a conventional swelling meter of wet type, which is used for silver halide photosensitive photographic materials. Specifically, there can be used the methods disclosed in Japanese Patent Publication (Kokoku, hereinafter referred to as JP-B) 5-22903, JP-A-7-270962, JP-A-8-76303, JP-A-8-240877, U.S. Pat. Nos. 3,841,872 and 5,561,038, provided that the saturation swelling time should be obtained as follows. That is, a photothermographic material is conditioned for moisture content at 30° C. and relative humidity of 40% for 1 day, then a predetermined amount of distilled water at 21° C. is dropped onto the surface of the photothermographic material on the image-forming layer side, and time that is required until a swelling value reaches 90% of final constant swelling value is measured to obtain the saturation swelling time.

The object of the present invention is to lower the humidity dependency of developed character line width. This phenomenon of the humidity dependency of developed character line width is not observed in the conventional photosensitive photographic materials of wet type for use in printing, and the phenomenon is characteristic for photothermographic materials utilizing heat development, in particular, photothermographic materials utilizing nucleating agents.

The saturation swelling time of the photothermographic materials can be controlled by several kinds of means. For example, the saturation swelling time of a photothermographic material to be produced can be controlled by varying liquid film surface temperature when the image-forming layer or protective layer is coated on a support. In this case, a higher liquid film surface temperature provides a longer saturation swelling time of the photothermographic material. Alternatively, by varying a coating amount of latex solid content or film thickness of a protective layer (preferably the protective layer remotest from the support), the saturation swelling time of a photothermographic material to be produced can also be controlled. In this case, an increased coating amount of latex solid content or film thickness provides a longer saturation swelling time.

The photothermographic material of the present invention contains a non-photosensitive silver salt of an organic acid. The non-photosensitive silver salt of an organic acid that can be used in the present invention is a silver salt relatively stable against light, but forms a silver image when it is heated at 80° C. or higher in the presence of an exposed photocatalyst (e.g., a latent image of photosensitive silver halide) and a reducing agent. The silver salt of an organic acid may be any organic substance containing a source of reducible silver ions. Silver salts of an organic acid, in particular, silver salts of a long chained aliphatic carboxylic acid having from 10 to 30, preferably from 15 to 28 carbon atoms, are preferred. Complexes of organic or inorganic acid silver salts of which ligands have a complex stability constant in the range of 4.0–10.0 are also preferred. The silver supplying substance can preferably constitute about 5–70 weight % of the image-forming layer. Preferred examples of the silver salts of an organic acid include silver salts of organic compounds having carboxyl group. Specifically, the silver salts of an organic acid may be silver salts of an aliphatic carboxylic acid and silver salts of an aromatic carboxylic acid, but not limited to these. Preferred examples

of the silver salts of an aliphatic carboxylic acid include silver behenate, silver arachidinate, silver stearate, silver oleate, silver laurate, silver caproate, silver myristate, silver palmitate, silver maleate, silver fumarate, silver tartrate, silver linoleate, silver butyrate, silver camphorate, mixtures thereof and so forth.

In the present invention, there is preferably used silver salt of an organic acid having a silver behenate content of 75 mole % or more, more preferably silver salt of an organic acid having a silver behenate content of 85 mole % or more, among the aforementioned silver salts of an organic acid and mixtures of silver salts of an organic acid. The silver behenate content used herein means a molar percent of silver behenate with respect to silver salt of an organic acid to be used. As silver salts of an organic acid other than silver behenate contained in the silver salts of organic acid used for the present invention, the silver salts of an organic acid exemplified above can preferably be used.

Silver salts of an organic acid that can be preferably used in the present invention can be prepared by allowing a solution or suspension of an alkali metal salt (e.g., Na salts, K salts, Li salts) of the aforementioned organic acids to react with silver nitrate. As the preparation method, the method described in Japanese Patent Application No. 11-104187, paragraphs 0019-0021 can be used.

In the present invention, a method of preparing a silver salt of an organic acid by adding an aqueous solution of silver nitrate and a solution of alkali metal salt of an organic acid to a sealable means for mixing liquids can preferably be used. Specifically, the method described in Japanese Patent Application No. 11-203413 can be used.

In the present invention, a dispersing agent soluble in water can be added to the aqueous solution of silver nitrate and the solution of alkali metal salt of an organic acid or reaction mixture. Type and amount of the dispersing agent used in this case are specifically mentioned in Japanese Patent Application No. 11-115457, paragraph 0052.

The silver salt of an organic acid for use in the present invention is preferably prepared in the presence of a tertiary alcohol. The tertiary alcohol preferably has a total carbon number of 15 or less, more preferably 10 or less. Examples of preferred tertiary alcohols include tert-butanol. However, tertiary alcohol that can be used for the present invention is not limited to it.

The tertiary alcohol for use in the present invention may be added in any timing during the preparation of the organic acid silver salt, but the tertiary alcohol is preferably used by adding at the time of preparation of the organic acid alkali metal salt to dissolve the organic alkali metal salt. The tertiary alcohol for use in the present invention may be added in any amount of from 0.01 to 10 in terms of the weight ratio to water used as a solvent at the preparation of the silver salt of an organic acid, but preferably added in an amount of from 0.03 to 1 in terms of weight ratio to water.

Although shape and size of the organic acid silver salt are not particularly limited, those mentioned in Japanese Patent Application No. 11-104187, paragraph 0024 can be preferably used. The shape of the organic acid silver salt can be determined from a transmission electron microscope image of organic silver salt dispersion. An example of the method for determining monodispersibility is a method comprising obtaining the standard deviation of a volume weight average diameter of the organic acid silver salt. The percentage of a value obtained by dividing the standard deviation by the volume weight average diameter (variation coefficient) is preferably 80% or less, more preferably 50% or less, par-

ticularly preferably 30% or less. As a measurement method, for example, the grain size can be determined by irradiating organic acid silver salt dispersed in a solution with a laser ray and determining an autocorrelation function for change of the fluctuation of the scattered light with time (volume weight average diameter). The average grain size determined by this method is preferably from 0.05 to 10.0  $\mu\text{m}$ , more preferably from 0.1 to 5.0  $\mu\text{m}$ , further preferably from 0.1 to 2.0  $\mu\text{m}$ , as in solid microparticle dispersion.

10 The silver salt of an organic acid that can be used in the present invention is preferably desalts. The desalting method is not particularly limited and any known methods may be used. Known filtration methods such as centrifugal filtration, suction filtration, ultrafiltration and flocculation 15 washing by coagulation may be preferably used. As the method of ultrafiltration, the method described in Japanese Patent Application No. 11-115457 can be used.

For obtaining an organic acid silver salt solid dispersion having a high S/N ratio and a small grain size and being free 20 from coagulation, there is preferably used a dispersion method comprising steps of converting an aqueous dispersion that contains a silver salt of an organic acid as an image-forming medium and contains substantially no photosensitive silver salt into a high-speed flow dispersion, and 25 then releasing the pressure. As such a dispersion method, the method mentioned in Japanese Patent Application No. 11-104187, paragraphs 0027-0038 can be used.

The grain size distribution of the silver salt of an organic acid preferably corresponds to monodispersion. Specifically, 30 the percentage (variation coefficient) of the value obtained by dividing the standard deviation by the volume weight average diameter is preferably 80% or less, more preferably 50% or less, particularly preferably 30% or less.

35 The organic acid silver salt grain solid dispersion used for the present invention consists at least of a silver salt of an organic acid and water. While the ratio of the silver salt of an organic acid and water is not particularly limited, the ratio of the silver salt of an organic acid is preferably in the range of 5-50 weight %, particularly preferably 10-30 weight %, 40 with respect to the total weight. While it is preferred that the aforementioned dispersing agent should be used, it is preferably used in a minimum amount within a range suitable for minimizing the grain size, and it is preferably used in an amount of 0.5-30 weight %, particularly preferably 1-15 weight %, with respect to the silver salt of an organic acid.

The silver salt of an organic acid for use in the present invention may be used in any desired amount. However, it is preferably used in an amount of from 0.1 to 5 g/m<sup>2</sup>, more 50 preferably from 1 to 3 g/m<sup>2</sup>, in terms of silver.

In the present invention, metal ions selected from Ca, Mg, Zn and Ag are preferably added to the non-photosensitive silver salt of an organic acid. The metal ions selected from Ca, Mg, Zn and Ag are preferably added to the non-photosensitive silver salt of an organic acid in the form of a water-soluble metal salt, not a halide compound. Specifically, they are preferably added in the form of nitrate or sulfate. Addition of halide is not preferred, since it degrades image storability, i.e., so-called printing-out 55 property, of the photosensitive material against light (indoor light, sun light etc.) after the development. Therefore, in the present invention, it is preferable to add the ions in the form of water-soluble metal salts, which are not the aforementioned halide compound.

60 The metal ions selected from Ca, Mg, Zn and Ag, which are preferably used in the present invention, may be added any time after the formation of non-photosensitive organic

acid silver salt grains and immediately before the coating operation, for example, immediately after the formation of grains, before dispersion, after dispersion, before and after the formation of coating solution and so forth. They are preferably added after dispersion, or before or after the formation of coating solution.

In the present invention, the metal ions selected from Ca, Mg, Zn and Ag are preferably added in an amount of  $10^{-3}$  to  $10^{-1}$  mole, particularly  $5 \times 10^{-3}$  to  $5 \times 10^{-2}$  mole, per one mole of non-photosensitive silver salt of an organic acid.

The photothermographic material of the present invention contains a photosensitive silver halide. The photosensitive silver halide used for the present invention is not particularly limited as for the halogen composition, and silver chloride, silver chlorobromide, silver bromide, silver iodobromide, silver chloroiodobromide and so forth may be used. As for the preparation of grains of the photosensitive silver halide emulsion, the grains can be prepared by the method described in JP-A-11-119374, paragraphs 0127-0224. However, the method is not particularly limited to this method.

Examples of the form of silver halide grains include a cubic form, octahedral form, tetradecahedral form, tabular form, spherical form, rod-like form, potato-like form and so forth. In particular, cubic grains and tabular grains are preferred for the present invention. As for the characteristics of the grain form such as aspect ratio and surface index of the grains, they may be similar to those described in JP-A-11-119374, paragraph 0225. Further, the halide composition may have a uniform distribution in the grains, or the composition may change stepwise or continuously in the grains. Silver halide grains having a core/shell structure may also be preferably used. Core/shell grains having preferably a double to quintuple structure, more preferably a double to quadruple structure may be used. A technique for localizing silver bromide on the surface of silver chloride or silver chlorobromide grains may also be preferably used.

As for the grain size distribution of the silver halide grains used in the present invention, the grains show monodispersion degree of 30% or less, preferably 1-20%, more preferably 5-15%. The monodispersion degree used herein is defined as a percentage (%) of a value obtained by dividing standard deviation of grain size by average grain size (variation coefficient). The grain size of the silver halide grains is represented as a ridge length for cubic grains, or a diameter as circle of projected area for the other grains (octahedral grains, tetradecahedral grains, tabular grains and so forth) for convenience.

The photosensitive silver halide grains preferably contain a metal of Group VII or Group VIII in the periodic table of elements or a complex of such a metal. The metal or the center metal of the complex of a metal of Group VII or Group VIII of the periodic table is preferably rhodium, rhenium, ruthenium, osmium or iridium. Particularly preferred metal complexes are  $(\text{NH}_4)_3\text{Rh}(\text{H}_2\text{O})\text{Cl}_5$ ,  $\text{K}_2\text{Ru}(\text{NO})\text{Cl}_5$ ,  $\text{K}_3\text{IrCl}_6$  and  $\text{K}_4\text{Fe}(\text{CN})_6$ . The metal complexes may be used each alone, or two or more complexes of the same or different metals may also be used in combination. The metal complex content is preferably from  $1 \times 10^{-9}$  to  $1 \times 10^{-3}$  mole, more preferably  $1 \times 10^{-8}$  to  $1 \times 10^{-4}$  mole, per mole of silver. As for specific structures of metal complexes, metal complexes of the structures described in JP-A-7-225449 and so forth can be used. Types and addition methods of these heavy metals and complexes thereof are described in JP-A-11-119374, paragraphs 0227-0240.

The photosensitive silver halide grains may be desalted by washing methods with water known in the art, such as the

noodle washing and flocculation. However, the grain may not be desalted in the present invention.

The photosensitive silver halide grains are preferably subjected to chemical sensitization. For the chemical sensitization, the method described in JP-A-11-119374, paragraphs 0242-0250 can preferably be used.

Silver halide emulsions used in the present invention may be added with thiosulfonic acid compounds by the method described in EP-A-293917.

As gelatin used with the photosensitive silver halide used in the present invention, low molecular weight gelatin is preferably used in order to maintain good dispersion state of the silver halide emulsion in a coating solution containing a silver salt of an organic acid. The low molecular weight gelatin has a molecular weight of 500-60,000, preferably 1,000-40,000. While such low molecular weight gelatin may be added during the formation of grains or dispersion operation after the desalting treatment, it is preferably added during dispersion operation after the desalting treatment. It is also possible to use ordinary gelatin (molecular weight of about 100,000) during the grain formation and use low molecular gelatin during dispersion operation after the desalting treatment.

While the concentration of dispersion medium may be 0.05-20 weight %, it is preferably in the range of 5-15 weight % in view of handling. As for type of gelatin, alkali-treated gelatin is usually used. Besides that, however, acid-treated gelatin, modified gelatin such as phthalated gelatin and so forth can also be used.

In the photosensitive material used for the present invention, one kind of photosensitive silver halide emulsion may be used or two or more different emulsions (for example, those having different average grain sizes, different halogen compositions, different crystal habits or those subjected to chemical sensitization under different conditions) may be used in combination.

The amount of the photosensitive silver halide per mole of the silver salt of an organic acid is preferably from 0.01-0.5 mole, more preferably from 0.02-0.3 mole, still more preferably from 0.03-0.25 mole. Methods and conditions for mixing photosensitive silver halide and silver salt of an organic acid, which are prepared separately, are not particularly limited so long as the effect of the present invention can be attained satisfactorily. Examples thereof include, for example, a method of mixing silver halide grains and silver salt of an organic acid after completion of respective preparations by using a high-speed stirring machine, ball mill, sand mill, colloid mill, vibrating mill, homogenizer or the like, or a method of preparing a silver salt of an organic acid with mixing a photosensitive silver halide obtained separately at any time during the preparation of the silver salt of an organic acid. For the mixing of them, mixing two or more kinds of aqueous dispersions of the silver salt of an organic acid and two or more kinds of aqueous dispersions of the photosensitive silver salt is preferably used for controlling photographic properties.

As a sensitizing dye that can be used for the present invention, there can be advantageously selected those sensitizing dyes that can spectrally sensitize silver halide grains within a desired wavelength range after they are adsorbed by the silver halide grains and have spectral sensitivity suitable for spectral characteristics of the light source to be used for exposure. For example, as dyes that spectrally sensitize in a wavelength range of 550 nm to 750 nm, there can be mentioned the compounds of formula (II) described in JP-A-10-186572, and more specifically, dyes of II-6, II-7,

II-14, II-15, II-18, II-23 and II-25 mentioned in the same can be exemplified as preferred dyes. As dyes that spectrally sensitize in a wavelength range of 750 nm to 1400 nm, there can be mentioned the compounds of formula (I) described in JP-A-11-119374, and more specifically, dyes of (25), (26), (30) (32), (36), (37), (41), (49) and (54) mentioned in the same can be exemplified as preferred dyes. Further, as dyes forming J-band, those disclosed in U.S. Pat. Nos. 5,510,236, 3,871,887 (Example 5), JP-A-2-96131 and JP-A-59-48753 can be exemplified as preferred dyes. These sensitizing dyes can be used each alone, or two or more of them can be used in combination.

These sensitizing dyes can be added by the method described in JP-A-11-119374, paragraph 0106. However, the method is not particularly limited to this method.

While the amount of the sensitizing dye used in the present invention may be selected to be a desired amount depending on the performance including sensitivity and fog, it is preferably used in an amount of  $10^{-6}$ –1 mole, more preferably  $10^{-4}$ – $10^{-1}$  mole, per mole of silver halide in the photosensitive layer.

In the present invention, supersensitizers can be used in order to improve spectral sensitization efficiency. Examples of the supersensitizer used for the present invention include the compounds disclosed in EP-A-587338, U.S. Pat. Nos. 3,877,943 and 4,873,184, and compounds selected from heteroaromatic or aliphatic mercapto compounds, heteroaromatic disulfide compounds, stilbenes, hydrazines and triazines, and so forth.

Particularly preferred supersensitizers are heteroaromatic mercapto compounds and heteroaromatic disulfide compounds disclosed in JP-A-5-341432, the compounds represented by the formulas (I) and (II) mentioned in JP-A-4-182639, stilbene compounds represented by the formula (I) mentioned in JP-A-10-111543 and the compounds represented by the formula (I) mentioned in JP-A-11-109547. Specifically, there can be mentioned the compounds of M-1 to M-24 mentioned in JP-A-5-341432, the compounds of d-1) to d-14) mentioned in JP-A-4-182639, the compounds of SS-01 to SS-07 mentioned in JP-A-10-111543 and the compounds of 31, 32, 37, 38, 41–45 and 51–53 mentioned in JP-A-11-109547.

These supersensitizers can be added to the emulsion layer preferably in an amount of  $10^{-4}$ –1 mole, more preferably in an amount of 0.001–0.3 mole per mole of silver halide.

The photothermographic material of the present invention contains a nucleating agent. While type of the nucleating agent that can be used in the present invention is not particularly limited, examples thereof include all of the hydrazine derivatives represented by the formula (H) mentioned in Japanese Patent Application No. 11-87297 (specifically, the hydrazine derivatives mentioned in Tables 1–4 of the same), the hydrazine derivatives described in JP-A-10-10672, JP-A-10-161270, JP-A-10-62898, JP-A-9-304870, JP-A-9-304872, JP-A-9-304871, JP-A-10-31282, U.S. Pat. No. 5,496,695 and EP-A-741320.

Particularly preferably used nucleating agents are the substituted alkene derivatives, substituted isoxazole derivatives and particular acetal compounds represented by the formulas (1) to (3) mentioned in Japanese Patent Application No. 11-87297, and more preferably, the cyclic compounds represented by the formula (A) or (B) mentioned in the same, specifically Compounds 1–72 mentioned in Chem. 8 to Chem. 12 of the same may be used. Two or more of these nucleating agents may be used in combination.

The nucleating agent may be used after being dissolved in an appropriate organic solvent such as alcohols (e.g.,

methanol, ethanol, propanol, fluorinated alcohol), ketones (e.g., acetone, methyl ethyl ketone), dimethylformamide, dimethyl sulfoxide or methyl cellosolve.

Further, it may also be used as an emulsion dispersion mechanically prepared according to an already well known emulsion dispersion method by using an oil such as dibutyl phthalate, tricresyl phosphate, glyceryl triacetate or diethyl phthalate, ethyl acetate or cyclohexanone as an auxiliary solvent for dissolution. Alternatively, the nucleating agent may be used by dispersing powder of the nucleating agent in a suitable solvent such as water using a ball mill, colloid mill, or by means of ultrasonic wave according to a known method for solid dispersion.

While the nucleating agent may be added to any layer on the image-forming layer side, it is preferably added to the image-forming layer or a layer adjacent thereto.

The amount of the nucleating agent is  $1 \times 10^{-6}$  mole to 1 mole, more preferably from  $1 \times 10^{-5}$  mole to  $5 \times 10^{-1}$  mole, further preferably from  $2 \times 10^{-5}$  mole to  $2 \times 10^{-1}$  mole, per mole of silver.

In addition to the aforementioned compounds, the compounds disclosed in U.S. Pat. Nos. 5,545,515, 5,635,339, 5,654,130 and 5,686,228, and International Patent Publication WO97/34196, and the compounds disclosed in JP-A-11-119372, JP-A-11-133546, JP-A-11-119373, JP-A-11-109546, JP-A-11-95365, JP-A-11-95366 and JP-A-11-149136 may also be used.

In the present invention, a contrast accelerator may be used in combination with the above-described nucleating agent for the formation of an ultrahigh contrast image. For example, amine compounds described in U.S. Pat. No. 5,545,505, specifically, AM-1 to AM-5; hydroxamic acids described in U.S. Pat. No. 5,545,507, specifically, HA-1 to HA-11; acrylonitriles described in U.S. Pat. No. 5,545,507, specifically, CN-1 to CN-13; hydrazine compounds described in U.S. Pat. No. 5,558,983, specifically, CA-1 to CA-6; and onium salts described in JP-A-9-297368, specifically, A-1 to A-42, B-1 to B-27 and C-1 to C-14 and so forth may be used.

Formic acid and formic acid salts serve as a strongly fogging substance in a photothermographic material containing a non-photosensitive silver salt, a photosensitive silver halide and a binder. In the present invention, the photothermographic material preferably contains formic acid or a formic acid salt on the side having the image-forming layer containing a photosensitive silver halide in an amount of 5 mmol or less, more preferably 1 mmol or less, per 1 mole of silver.

In the photothermographic material the present invention, an acid formed by hydration of diphosphorus pentoxide or a salt thereof is preferably used together with the nucleating agent. Examples of the acid formed by hydration of diphosphorus pentoxide or a salt thereof include metaphosphoric acid (salt), pyrophosphoric acid (salt), orthophosphoric acid (salt), triphosphoric acid (salt), tetraphosphoric acid (salt), hexametaphosphoric acid (salt) and so forth. Particularly preferably used acids formed by hydration of diphosphorus pentoxide or salts thereof are orthophosphoric acid (salt) and hexametaphosphoric acid (salt). Specific examples of the salt are sodium orthophosphate, sodium hexametaphosphate, ammonium hexametaphosphate and so forth.

The acid formed by hydration of diphosphorus pentoxide or a salt thereof that can be preferably used in the present invention is added to the image-forming layer or a binder layer adjacent thereto in order to obtain the desired effect with a small amount of the acid or a salt thereof.

## 11

The acid formed by hydration of diphosphorus pentoxide or a salt thereof may be used in a desired amount (coated amount per m<sup>2</sup> of the photosensitive material) depending on the desired performance including sensitivity and fog. However, it can preferably be used in an amount of 0.1–500 mg/m<sup>2</sup>, more preferably 0.5–100 mg/m<sup>2</sup>.

The photothermographic material of the present invention preferably contains a reducing agent for the silver salt of an organic acid. The reducing agent for the silver salt of an organic acid may be any substance that reduces silver ion to metal silver, preferably such an organic substance. Conventional photographic developers such as phenidone, hydroquinone and catechol are useful, but a hindered phenol reducing agent is preferred. The reducing agent is preferably contained in an amount of from 5 to 50 mole %, more preferably from 10 to 40 mole %, per mole of silver on the side having the image-forming layer. The reducing agent may be added to any layer on the side having an image-forming layer. In the case of adding the reducing agent to a layer other than the image-forming layer, the reducing agent is preferably used in a slightly large amount of from 10–50 mole % per mole of silver. The reducing agent may also be a so-called precursor that is derived to effectively function only at the time of development.

For photothermographic materials using silver salt of an organic acid, reducing agents of a wide range can be used. There can be used, for example, the reducing agents disclosed in JP-A-46-6074, JP-A-47-1238, JP-A-47-33621, JP-A-49-46427, JP-A-49-115540, JP-A-50-14334, JP-A-50-36110, JP-A-50-147711, JP-A-51-32632, JP-A-51-1023721, JP-A-51-32324, JP-A-51-51933, JP-A-52-84727, JP-A-55-108654, JP-A-56-146133, JP-A-57-82828, JP-A-57-82829, JP-A-6-3793, U.S. Pat. Nos. 3,679,426, 3,751, 252, 3,751,255, 3,761,270, 3,782,949, 3,839,048, 3,928,686 and 5,464,738, German Patent No. 2,321,328, EP-A-692732 and so forth. Examples thereof include amidoximes such as phenylamidoxime, 2-thienylamidoxime and p-phenoxyphenylamidoxime; azines such as 4-hydroxy-3,5-dimethoxybenzaldehyde azine; combinations of an aliphatic carboxylic acid arylhydrazide with ascorbic acid such as a combination of 2,2-bis(hydroxymethyl)propionyl-β-phenylhydrazine with ascorbic acid; combinations of polyhydroxybenzene with hydroxylamine, reductone and/or hydrazine such as a combination of hydroquinone with bis(ethoxyethyl)hydroxylamine, piperidinohexose reductone or formyl-4-methylphenylhydrazine; hydroxamic acids such as phenylhydroxamic acid, p-hydroxyphenylhydroxamic acid and β-anilinehydroxamic acid; combinations of an azine with a sulfonamidophenol such as a combination of phenothiazine with 2,6-dichloro-4-benzenesulfonamidophenol; α-cyanophenylacetic acid derivatives such as ethyl-α-cyano-2-methylphenylacetate and ethyl-α-cyanophenylacetate; bis-β-naphthols such as 2,2'-dihydroxy-1,1'-binaphthyl, 6,6'-dibromo-2,2'-dihydroxy-1,1'-binaphthyl and bis(2-hydroxy-1-naphthyl)methane; combinations of a bis-β-naphthol with a 1,3-dihydroxybenzene derivative (e.g., 2,4-dihydroxybenzophenone, 2',4'-dihydroxyacetophenone); 5-pyrazolones such as 3-methyl-1-phenyl-5-pyrazolone; reductones such as dimethylaminohexose reductone, anhydriodihydroaminohexose reductone and anhydriodihydropiperidonehexose reductone; sulfonamidophenol reducing agents such as 2,6-dichloro-4-benzenesulfonamidophenol and p-benzenesulfonamidophenol; 2-phenylindane-1,3-diones; chromans such as 2,2-dimethyl-7-t-butyl-6-hydroxychroman; 1,4-dihydropyridines such as 2,6-dimethoxy-3,5-dicarboethoxy-1,4-dihydropyridine;

## 12

bisphenols such as bis(2-hydroxy-3-t-butyl-5-methylphenyl)methane, 2,2-bis(4-hydroxy-3-methylphenyl)propane, 4,4-ethylidene-bis(2-t-butyl-6-methylphenol), 1,1-bis(2-hydroxy-3,5-dimethylphenyl)-3,5,5-trimethylhexane and 2,2-bis(3,5-dimethyl-4-hydroxyphenyl)propane; ascorbic acid derivatives such as 1-ascorbyl palmitate and ascorbyl stearate; aldehydes and ketones such as benzyl and biacetyl; 3-pyrazolidone and a certain kind of indane-1,3-diones; and chromanols such as tocopherol. Particularly preferred reducing agents are bisphenols and chromanols.

When the reducing agent is used in the present invention, it may be added in any form of an aqueous solution, solution in an organic solvent, powder, solid microparticle dispersion, emulsion dispersion or the like. The solid microparticle dispersion is performed by using a known pulverizing means (e.g., ball mill, vibrating ball mill, sandmill, colloidmill, jetmill, roller mill). At the time of solid microparticle dispersion, a dispersion aid may also be used.

When an additive known as a “toning agent” capable of improving the image is added, the optical density increases in some cases. The toning agent may also be advantageous in forming a black silver image depending on the case. The toning agent is preferably contained in a layer on the side having the image-forming layer in an amount of from 0.1–50 mole %, more preferably from 0.5–20 mole %, per mole of silver. The toning agent may be a so-called precursor that is derived to effectively function only at the time of development.

For the photothermographic material using a silver salt of an organic acid, toning agents of a wide range can be used. For example, there can be used toning agents disclosed in JP-A-46-6077, JP-A-47-10282, JP-A-49-5019, JP-A-49-5020, JP-A-49-91215, JP-A-49-91215, JP-A-50-2524, JP-A-50-32927, JP-A-50-67132, JP-A-50-67641, JP-A-50-114217, JP-A-51-3223, JP-A-51-27923, JP-A-52-14788, JP-A-52-99813, JP-A-53-1020, JP-A-53-76020, JP-A-54-156524, JP-A-54-156525, JP-A-61-183642, JP-A-4-56848, JP-B-49-10727, JP-B-54-20333, U.S. Pat. Nos. 3,080,254, 3,446,648, 3,782,941, 4,123,282 and 4,510,236, British Patent No. 1,380,795, Belgian Patent No. 841910 and so forth. Specific examples of the toning agent include phthalimide and N-hydroxyphthalimide; succinimide, pyrazolin-5-ones and cyclic imides such as quinazolinone, 3-phenyl-2-pyrazolin-5-one, 1-phenylurazole, quinazoline and 2,4-thiazolidinedione; naphthalimides such as N-hydroxy-1,8-naphthalimide; cobalt complexes such as cobalt hexaminetrifluoroacetate; mercaptanes such as 3-mercaptop-1,2,4-triazole, 2,4-dimercaptopyrimidine, 3-mercaptop-4,5-diphenyl-1,2,4-triazole and 2,5-dimercapto-1,3,4-thiadiazole; N-(aminomethyl)aryldicarboxyimides such as N,N-(dimethylaminomethyl)phthalimide and N,N-(dimethylaminomethyl)naphthalene-2,3-dicarboxyimide; blocked pyrazoles, isothiuronium derivatives and a certain kind of photobleaching agents such as N,N'-hexamethylenebis(1-carbamoyl-3,5-dimethylpyrazole), 1,8-(3,6-diazaoctane)bis(isothiuroniumtrifluoroacetate) and 2-(tribromomethylsulfonyl)benzothiazole; 3-ethyl-5-[(3-ethyl-2-benzothiazolinylidene)-1-methylethylidene]-2-thio-2,4-oxazolidinedione; phthalazinone, phthalazinone derivatives and metal salts thereof, such as 4-(1-naphthyl)phthalazinone, 6-chlorophthalazinone, 5,7-dimethoxyphthalazinone or 2,3-dihydro-1,4-phthalazinedione; combinations of phthalazinone with a phthalic acid derivative (e.g., phthalic acid, 4-methylphthalic acid, 4-nitrophthalic acid, tetrachlorophthalic acid anhydride); phthalazine, phthalazine derivatives (e.g., 4-(1-naphthyl)phthalazine, 6-chlorophthalazine,

13

5,7-dimethoxyphthalazine, 6-isobutyl-phthalazine, 6-tert-butylphthalazine, 5,7-dimethylphthalazine, 2,3-dihydrophthalazine) and metal salts thereof; combinations of a phthalazine or derivative thereof and a phthalic acid derivative (e.g., phthalic acid, 4-methylphthalic acid, 4-nitrophthalic acid, tetrachlorophthalic acid anhydride); quinazolinedione, benzoxazine and naphthoxazine derivatives; rhodium complexes which function not only as a toning agent but also as a halide ion source for the formation of silver halide at the site, such as ammonium hexachlororhodate(III), rhodium bromide, rhodium nitrate and potassium hexachlororhodate(III); inorganic peroxides and persulfates such as ammonium disulfide peroxide and hydrogen peroxide; benzoxazine-2,4-diones such as 1,3-benzoxazin-2,4-dione, 8-methyl-1,3-benzoxazin-2,4-dione and 6-nitro-1,3-benzoxazin-2,4-dione; pyrimidines and asymmetric triazines such as 2,4-dihydroxypyrimidine and 2-hydroxy-4-aminopyrimidine; azauracil and tetraazapentalene derivatives such as 3,6-dimercapto-1,4-diphenyl-1H, 4H-2,3a,5,6a-tetraazapentalene and 1,4-di(o-chlorophenyl)-3,6-dimercapto-1H,4H-2,3a,5,6a-tetraazapentalene and so forth.

In the present invention, the phthalazine derivatives represented by the general formula (F) mentioned in JP-A-2000-35631 are preferably used as the toning agent. Specifically, A-1 to A-10 mentioned in the same are preferably used.

The toning agent may be added in any form of a solution, powder, solid microparticle dispersion or the like. The solid microparticle dispersion is performed by using a known pulverization means (e.g., ball mill, vibrating ball mill, sand mill, colloid mill, jet mill, roller mill). At the time of solid microparticle dispersion, a dispersion aid may also be used.

The photothermographic material of the present invention preferably has a film surface pH of 6.0 or less, more preferably 5.5 or less before heat development. While it is not particularly limited as for the lower limit, it is normally around 3 or higher.

For controlling the film surface pH, an organic acid such as phthalic acid derivatives or a nonvolatile acid such as sulfuric acid, and a volatile base such as ammonia are preferably used to lower the film surface pH. In particular, ammonia is preferred to achieve a low film surface pH, because it is highly volatile and therefore it can be removed before coating or heat development. A method for measuring the film surface pH is described in Japanese Patent Application No. 11-87297, paragraph 0123.

The silver halide emulsion and/or the silver salt of an organic acid for use in the photothermographic material of the present invention can be further prevented from the production of additional fog or stabilized against the reduction in sensitivity during the stock storage, by an antifoggant, a stabilizer or a stabilizer precursor. Examples of suitable antifoggant, stabilizer and stabilizer precursor that can be used individually or in combination include thiazonium salts described in U.S. Pat. Nos. 2,131,038 and 2,694,716, azaindenes described in U.S. Pat. Nos. 2,886,437 and 2,444,605, mercury salts described in U.S. Pat. No. 2,728,663, urazoles described in U.S. Pat. No. 3,287,135, sulfocatechols described in U.S. Pat. No. 3,235,652, oximes, nitrons and nitroindazoles described in British Patent No. 623,448, polyvalent metal salts described in U.S. Pat. No. 2,839,405, thiuronium salts described in U.S. Pat. No. 3,220,839, palladium, platinum and gold salts described in U.S. Pat. Nos. 2,566,263 and 2,597,915, halogen-substituted organic compounds described in U.S. Pat. Nos. 4,108,665

14

and 4,442,202, triazines described in U.S. Pat. Nos. 4,128,557, 4,137,079, 4,138,365 and 4,459,350, phosphorus compounds described in U.S. Pat. No. 4,411,985 and so forth.

The photothermographic material of the present invention may contain a benzoic acid compound for the purpose of achieving high sensitivity or preventing fog. The benzoic acid compound for use in the present invention may be any benzoic acid derivative, but preferred examples thereof include the compounds described in U.S. Pat. Nos. 4,784,939 and 4,152,160 and JP-A-9-329863, JP-A-9-329864 and JP-A-9-281637. The benzoic acid compound for use in the present invention may be added to any layer of the photothermographic material, but the layer to which the benzoic acid is added is preferably a layer on the surface having the image-forming layer, more preferably a layer containing a silver salt of an organic acid. The benzoic acid compound for use in the present invention may be added at any step during the preparation of the coating solution. In the case of adding the benzoic acid compound to a layer containing a silver salt of an organic acid, it may be added at any step from the preparation of the silver salt of an organic acid to the preparation of the coating solution, but it is preferably added in the period after the preparation of the silver salt of an organic acid and immediately before the coating. The benzoic acid compound may be added in any form such as powder, solution, and microparticle dispersion, or may be added as a solution containing a mixture of the benzoic acid compound with other additives such as a sensitizing dye, reducing agent and toning agent. The benzoic acid compound may be added in any amount. However, the addition amount thereof is preferably from  $1 \times 10^{-6}$  to 2 mole, more preferably from  $1 \times 10^{-3}$  to 0.5 mole, per mole of silver.

Although not essential for practicing the present invention, it is advantageous in some cases to add a mercury(II) salt as an antifoggant to the image-forming layer. Preferred mercury(II) salts for this purpose are mercury acetate and mercury bromide. The addition amount of mercury for use in the present invention is preferably from  $1 \times 10^{-9}$  to  $1 \times 10^{-3}$  mole, more preferably from  $1 \times 10^{-8}$  to  $1 \times 10^{-4}$  mole, per mole of coated silver.

The antifoggant that is particularly preferably used in the present invention is an organic halide, and examples thereof include the compounds described in JP-A-50-119624, JP-A-50-120328, JP-A-51-121332, JP-A-54-58022, JP-A-56-70543, JP-A-56-99335, JP-A-59-90842, JP-A-61-129642, JP-A-62-129845, JP-A-6-208191, JP-A-7-5621, JP-A-7-2781, JP-A-8-15809 and U.S. Pat. Nos. 5,340,712, 5,369,000 and 5,464,737.

The hydrophilic organic halides represented by the formula (P) mentioned in Japanese Patent Application No. 11-87297 can be preferably used as the antifoggant. Specifically, the compounds (P-1) to (P-118) mentioned in the same are preferably used.

The amount of the organic halides is preferably  $1 \times 10^{-5}$  mole to 2 mole/mole Ag, more preferably  $5 \times 10^{-5}$  mole to 1 mole/mole Ag, further preferably  $1 \times 10^{-4}$  mole to  $5 \times 10^{-1}$  mole/mole Ag, in terms of molar amount per mole of Ag (mole/mole Ag). The organic halides may be used each alone, or two or more of them may be used in combination.

Further, the salicylic acid derivatives represented by the formula (Z) mentioned in Japanese Patent Application No. 11-87297 can be preferably used as the antifoggant. Specifically, the compounds (A-1) to (A-60) mentioned in the same are preferably used. The amount of the salicylic acid represented by the formula (Z) is preferably  $1 \times 10^{-5}$  mole to  $5 \times 10^{-1}$  mole/mole Ag, more preferably  $5 \times 10^{-5}$  mole

to  $1 \times 10^{-1}$  mole/mole Ag, further preferably  $1 \times 10^{-4}$  mole to  $5 \times 10^{-2}$  mole/mole Ag, in terms of molar amount per mole of Ag (mole/mole Ag). The salicylic acid derivatives may be used each alone, or two or more of them may be used in combination.

As antifoggants preferably used in the present invention, formalin scavengers are effective. Examples thereof include the compounds represented by the formula (S) and the exemplary compounds thereof (S-1) to (S-24) mentioned in Japanese Patent Application No. 11-23995.

The antifoggants used for the present invention may be used after being dissolved in an appropriate organic solvent such as alcohols (e.g., methanol, ethanol, propanol, fluorinated alcohol), ketones (e.g., acetone, methyl ethyl ketone), dimethylformamide, dimethyl sulfoxide or methyl cellosolve.

Further, they may also be used as an emulsion dispersion mechanically prepared according to an already well known emulsion dispersion method by using an oil such as dibutyl phthalate, tricresyl phosphate, glyceryl triacetate or diethyl phthalate, ethyl acetate or cyclohexanone as an auxiliary solvent for dissolution. Alternatively, they may be used by dispersing powder of them in a suitable solvent such as water using a ball mill, colloid mill, sand grinder mill, MANTON GAULIN, microfluidizer, or by means of ultrasonic wave according to a known method for solid dispersion.

While the antifoggants used in the present invention may be added to any layer on the image-forming layer side, that is, the image-forming layer or another layer on that side, they are preferably added to the image-forming layer or a layer adjacent thereto. The image-forming layer is a layer containing a reducible silver salt (silver salt of an organic acid), preferably such a image-forming layer further containing a photosensitive silver halide.

The photothermographic material of the present invention may contain a mercapto compound, disulfide compound or thione compound so as to control the development by inhibiting or accelerating the development or improve the storage stability before or after the development.

In the case of using a mercapto compound in the present invention, any structure may be used but those represented by Ar—SM or Ar—S—S—Ar are preferred, wherein M is a hydrogen atom or an alkali metal atom, and Ar is an aromatic ring or condensed aromatic ring containing one or more nitrogen, sulfur, oxygen, selenium or tellurium atoms. The heteroaromatic ring is preferably selected from benzimidazole, naphthimidazole, benzothiazole, naphthothiazole, benzoxazole, naphthoxazole, benzoselenazole, benzotellurazole, imidazole, oxazole, pyrazole, triazole, thiadiazole, tetrazole, triazine, pyrimidine, pyridazine, pyrazine, pyridine, purine, quinoline and quinazolinone. The heteroaromatic ring may have a substituent selected from, for example, the group consisting of a halogen (e.g., Br, Cl), hydroxy, amino, carboxy, alkyl (e.g., alkyl having one or more carbon atoms, preferably from 1 to 4 carbon atoms), alkoxy (e.g., alkoxy having one or more carbon atoms, preferably from 1 to 4 carbon atoms) and aryl (which may have a substituent). Examples of the mercapto substituted heteroaromatic compound include 2-mercaptopbenzimidazole, 2-mercaptopbenzoxazole, 2-mercaptopbenzothiazole, 2-mercaptop-5-methylbenzimidazole, 6-ethoxy-2-mercaptopbenzothiazole, 2,2'-dithiobis(benzothiazole), 3-mercaptop-1,2,4-triazole, 4,5-diphenyl-2-imidazolethiol, 2-mercaptopimidazole, 1-ethyl-2-mercaptopbenzimidazole, 2-mercaptopquinoline,

8-mercaptopurine, 2-mercaptop-4(3H)-quinazolinone, 7-trifluoromethyl-4-quinolinethiol, 2,3,5,6-tetrachloro-4-pyridinethiol, 4-amino-6-hydroxy-2-mercaptopurine monohydrate, 2-amino-5-mercaptop-1,3,4-thiadiazole, 3-amino-5-mercaptop-1,2,4-triazole, 4-hydroxy-2-mercaptopurine, 2-mercaptopurine, 4,6-di-amino-2-mercaptopurine, 2-mercaptop-4-methyl-purine hydrochloride, 3-mercaptop-5-phenyl-1,2,4-triazole, 1-phenyl-5-mercaptopurine, sodium 3-(5-mercaptopurine)benzenesulfonate, N-methyl-N'-(3-(5-mercaptopurine)phenyl)urea, 2-mercaptop-4-phenyloxazole and so forth. However, the present invention is not limited to these.

The amount of the mercapto compound is preferably from 0.0001 to 1.0 mole, more preferably from 0.001 to 0.3 mole, per mole of silver in the image-forming layer.

The photothermographic material of the present invention has an image-forming layer containing a silver salt of an organic acid, a reducing agent and a photosensitive silver halide on a support, and at least one protective layer is preferably provided on the image-forming layer. Further, the photothermographic material of the present invention preferably has at least one back layer on the side of the support opposite to the side of the image-forming layer (back surface), and polymer latex is used as binder of the image-forming layer, protective layer and back layer. The use of polymer latex for these layers enables coating with an aqueous system utilizing a solvent (dispersion medium) containing water as a main component. Not only this is advantageous for environment and cost, but also it makes it possible to provide photothermographic materials that generate no wrinkle upon heat development. Further, by using a support subjected to a predetermined heat treatment, there are provided photothermographic materials exhibiting little dimensional change in sizes before and after the heat development.

As the binder used for the present invention, the polymer latex explained below is preferably used.

Among image-forming layers containing a photosensitive silver halide in the photothermographic material of the present invention, at least one layer is preferably an image-forming layer utilizing polymer latex to be explained below in an amount of 50 weight % or more with respect to the total amount of binder. The polymer latex may be used not only in the image-forming layer, but also in the protective layer, back layer or the like. When the photothermographic material of the present invention is used for, in particular, printing use in which dimensional change causes problems, the polymer latex is preferably used also in a protective layer and a back layer. The term "polymer latex" used herein means a dispersion comprising hydrophobic water-insoluble polymer dispersed in a water-soluble dispersion medium as fine particles. The dispersed state may be one in which polymer is emulsified in a dispersion medium, one in which polymer underwent emulsion polymerization, emulsion dispersion, micelle dispersion, one in which polymer molecules having a hydrophilic portion are dispersed in molecular state or the like. Polymer latex used in the present invention is described in "Gosei Jushi Emulsion (Synthetic Resin Emulsion)", compiled by Taira Okuda and Hiroshi Inagaki, issued by Kobunshi Nankai (1978); "Gosei Latex no Oyo (Application of Synthetic Latex)", compiled by Takaaki Sugimura, Yasuo Kataoka, Souichi Suzuki and Keishi Kasahara, issued by Kobunshi Kankai (1993); Soichi Muroi, "Gosei Latex no Kagaku (Chemistry of Synthetic Latex)", Kobunshi Kankai (1970) and so forth. The dispersed particles preferably have an average particle

size of about 1–50000 nm, more preferably about 5–1000 nm. The particle size distribution of the dispersed particles is not particularly limited, and the particles may have either wide particle size distribution or monodispersed particle size distribution.

The polymer latex used in the present invention may be latex of the so-called core/shell type, which is different from ordinary polymer latex of a uniform structure. In this case, use of different glass transition temperatures of the core and shell may be preferred.

Preferred range of the glass transition temperature (Tg) of the polymer latex preferably used as the binder in the present invention varies for the protective layer, back layer and image-forming layer. As for the image-forming layer, the glass transition temperature is preferably –30 to 40° C. for accelerating diffusion of photographic elements during the heat development. Polymer latex used for the protective layer or back layer preferably has a glass transition temperature of 25 to 70° C., because these layers are brought into contact with various apparatuses.

The polymer latex used in the present invention preferably shows a minimum film forming temperature (MFT) of about –30–90° C., more preferably about 0–70° C. A film-forming aid may be added in order to control the minimum film forming temperature. The film-forming aid is also referred to as a plasticizer, and consists of an organic compound (usually an organic solvent) that lowers the minimum film forming temperature of the polymer latex. It is explained in, for example, the aforementioned Soichi Muroi, "Gosei Latex no Kagaku (Chemistry of Synthetic Latex)", Kobunshi Kanko Kai (1970).

Examples of polymer species used for the polymer latex used in the present invention include acrylic resins, polyvinyl acetate resins, polyester resins, polyurethane resins, rubber resins, polyvinyl chloride resins, polyvinylidene chloride resins and polyolefin resins, copolymers of monomers constituting these resins and so forth. The polymers may be linear, branched or crosslinked. They may be so-called homopolymers in which a single kind of monomer is polymerized, or copolymers in which two or more different kinds of monomers are polymerized. The copolymers may be random copolymers or block copolymers. The polymers may have a number average molecular weight of 5,000 to 1,000,000, preferably from 10,000 to 100,000. Polymers having a too small molecular weight may unfavorably suffer from insufficient mechanical strength of the image-forming layer, and those having a too large molecular weight may unfavorably suffer from bad film forming property.

Examples of the polymer latex used as the binder of the image-forming layer of the photothermographic material of the present invention include latex of methyl methacrylate/ethyl acrylate/methacrylic acid copolymer, latex of methyl methacrylate/butadiene/itaconic acid copolymer, latex of ethyl acrylate/methacrylic acid copolymer, latex of methyl methacrylate/2-ethylhexyl acrylate/styrene/acrylic acid copolymer, latex of styrene/butadiene/acrylic acid copolymer, latex of styrene/butadiene/divinylbenzene/methacrylic acid copolymer, latex of methyl methacrylate/vinyl chloride/acrylic acid copolymer, latex of vinylidene chloride/ethyl acrylate/acrylonitrile/methacrylic acid copolymer and so forth. More specifically, there can be mentioned latex of methyl methacrylate (33.5 weight %)/ethyl acrylate (50 weight %)/methacrylic acid (16.5 weight %) copolymer, latex of methyl methacrylate (47.5 weight %)/butadiene (47.5 weight %)/itaconic acid (5

weight %) copolymer, latex of ethyl acrylate (95 weight %)/methacrylic acid (5 weight %) copolymer and so forth. Such polymers are also commercially available and examples thereof include acrylic resins such as CEBIAN 5 A-4635, 46583, 4601 (all produced by Dicel Kagaku Kogyo Co., Ltd), Nipol Lx811, 814, 821, 820, 857 (all produced by Nippon Zeon Co., Ltd.), VONCORT R3340, R3360, R3370, 4280 (all produced by Dai-Nippon Ink & Chemicals, Inc.); polyester resins such as FINETEX ES650, 611, 675, 850 (all 10 produced by Dai-Nippon Ink & Chemicals, Inc.), WD-size and WMS (both produced by Eastman Chemical); polyurethane resins such as HYDRAN AP10, 20, 30, 40 (all produced by Dai-Nippon Ink & Chemicals, Inc.); rubber resins such as LACSTAR 7310K, 3307B, 4700H, 7132C (all 15 produced by Dai-Nippon Ink & Chemicals, Inc.) Nipol LX416, 410, 438C (all produced by Nippon Zeon Co., Ltd.); polyvinyl chloride resins such as G351, G576 (both produced by Nippon Zeon Co., Ltd.); polyvinylidene chloride resins such as L502, L513 (both produced by Asahi Chemical 20 Industry Co., Ltd.), ARON D7020, D504, D5071 (all produced by Mitsui Toatsu Co., Ltd.); and olefin resins such as CHEMPEARL S120 and SA100 (both produced by Mitsui Petrochemical Industries, Ltd.) and so forth. These polymers may be used individually or if desired, as a blend 25 of two or more of them.

The image-forming layer preferably contains 50 weight % or more, more preferably 70 weight % or more of the aforementioned polymer latex based on the total binder.

If desired, the image-forming layer may contain a hydrophilic polymer in an amount of 50 weight % or less of the total binder, such as gelatin, polyvinyl alcohol, methylcellulose, hydroxypropylcellulose, carboxymethylcellulose and hydroxypropylmethylcellulose. The amount of the hydrophilic polymer is preferably 30 weight % or less, more preferably 15 weight % or less, of the total binder in the image-forming layer.

The image-forming layer is preferably formed by coating an aqueous coating solution and then drying the coating solution. The term "aqueous" as used herein means that 40 water content of the solvent (dispersion medium) in the coating solution is 60 weight % or more. In the coating solution, the component other than water may be a water-miscible organic solvent such as methyl alcohol, ethyl alcohol, isopropyl alcohol, methyl cellosolve, ethyl cellosolve, dimethylformamide and ethyl acetate. Specific examples of the solvent composition include water/methanol=90/10, water/methanol=70/30, water/ethanol=90/10, water/isopropanol=90/10, water/dimethylformamide=95/5, water/methanol/dimethylformamide=80/15/5, and water/methanol/dimethylformamide=90/5/5 (the numerals indicate weight %).

The total amount of the binder in the image-forming layer is preferably from 0.2 to 30 g/m<sup>2</sup>, more preferably from 1 to 15 g/m<sup>2</sup>. The image-forming layer may contain a crosslinking agent for crosslinking, surfactant for improving coatability and so forth.

Further, a combination of polymer latexes having different I/O values is also preferably used as the binder of the protective layer. The I/O values are obtained by dividing an inorganicity value with an organicity values, both of which values are based on the organic conceptual diagram described in Japanese Patent Application No. 11-6872, paragraphs 0025–0029.

In the present invention, a plasticizer (e.g., benzyl alcohol, 2,2,4-trimethylpentanediol-1,3-monoisobutyrate etc.) described in Japanese Patent Application No.

11-143058, paragraphs 0021–0025 can be added to control the film-forming temperature. Further, a hydrophilic polymer may be added to a polymer binder, and a water-miscible organic solvent may be added to a coating solution as described in Japanese Patent Application No. 11-6872, paragraphs 0027–0028.

First polymer latex introduced with functional groups, and a crosslinking agent and/or second polymer latex having a functional group that can react with the first polymer latex, which are described in JP-A-2000-19678, paragraphs 0023–0041, can also be added to each layer.

The aforementioned functional groups may be carboxyl group, hydroxyl group, isocyanate group, epoxy group, N-methylol group, oxazolinyl group or the like. The crosslinking agent is selected from epoxy compounds, isocyanate compounds, blocked isocyanate compounds, methanolated compounds, hydroxy compounds, carboxyl compounds, amino compounds, ethylene-imine compounds, aldehyde compounds, halogen compounds and so forth. Specific examples of the crosslinking agent include, as isocyanate compounds, hexamethylene isocyanate, Duranate WB40-80D, WX-1741 (Asahi Chemical Industry Co., Ltd.), Bayhydur 3100 (Sumitomo Bayer Urethane Co., Ltd.), Takenate WD725 (Takeda Chemical Industries, Ltd.), Aquanate 100, 200 (Nippon Polyurethane Industry Co., Ltd.), water dispersion type polyisocyanates mentioned in JP-A-9-160172; as an amino compound, Sumitex Resin M-3 (Sumitomo Chemical Co., Ltd.); as an epoxy compound, Denacol EX-614B (Nagase Chemicals Ltd.); as a halogen compound, 2,4-dichloro-6-hydroxy-1,3,5-triazine sodium salt and so forth.

The total amount of the binders for the image-forming layer is preferably in the range of 0.2–30 g/m<sup>2</sup>, more preferably 1.0–15 g/m<sup>2</sup>.

The total amount of the binders for the protective layer is preferably in the range of 1–10.0 g/m<sup>2</sup>, more preferably 2–6.0 g/m<sup>2</sup>, as an amount required for attaining a film thickness of 3  $\mu\text{m}$  or more, which thickness is preferably used for the present invention.

The thickness of the protective layer preferably used for the present invention is 3  $\mu\text{m}$  or more, further preferably 4  $\mu\text{m}$  or more. Although the upper limit of the thickness of the protective layer is not particularly defined, the thickness is preferably 10  $\mu\text{m}$  or less, more preferably 8  $\mu\text{m}$  or less, in view of coating and drying.

The total amount of the binders for the back layer is preferably in the range of 0.01–10 g/m<sup>2</sup>, more preferably 0.05–5.0 g/m<sup>2</sup>.

Each of these layers may be provided as two or more layers. When the image-forming layer consists of two or more layers, it is preferred that polymer latex should be used as a binder for all of the layers. The protective layer is a layer provided on the image-forming layer, and it may consist of two or more layers. In such a case, it is preferred that polymer latex should be used for at least one layer, especially the outermost protective layer. Further, the back layer is a layer provided on an undercoat layer for the back surface of the support, and it may consist of two or more layers. In such a case, it is preferred that polymer latex should be used for at least one layer, especially the outermost back layer.

A lubricant referred to in the present specification means a compound which, when present at the surface of an object, reduces the friction coefficient of the surface compared with that observed when the compound is absent. The type of the lubricant is not particularly limited.

Examples of the lubricant that can be used in the present invention include the compounds described in JP-A-11-

84573, paragraphs 0061–0064 and Japanese Patent Application No. 11-106881, paragraphs 0049–0062.

Preferred examples of the lubricant include Cellosol 524 (main component: carnauba wax), Polylon A, 393, H-481 (main component: polyethylene wax), Himicron G-110 (main component: ethylene bisstearic acid amide), Himicron G-270 (main component: stearic acid amide) (all produced by Chukyo Yushi Co., Ltd.),

W-1:  $\text{C}_{16}\text{H}_{33}-\text{O}-\text{SO}_3\text{Na}$   
W-2:  $\text{C}_{18}\text{H}_{37}-\text{O}-\text{SO}_3\text{Na}$

and so forth.

The amount of the lubricant used is 0.1 to 50 weight %, preferably 0.5 to 30 weight %, of the amount of binder in a layer to which the lubricant is added.

When such a development apparatus as disclosed in Japanese Patent Application Nos. 11-346561 and 11-106881 is used, in which a photothermographic material is transported in a pre-heating section by facing rollers, and the material is transported in a heat development section by

driving force of rollers facing the image-forming layer side of the material, while the opposite back surface slides on a smooth surface, ratio of friction coefficients of the outermost surface of the image-forming layer side of the material and the outermost surface of the back layer is 1.5 or more.

Although the ratio is not particularly limited for its upper limit, it is about 30 or less. The value of  $\mu_b$  included in the following equation is 1.0 or less, preferably 0.05–0.8. The ratio can be obtained in accordance with the following equation. Ratio of friction coefficients=coefficient of

dynamic friction between roller material of heat development apparatus and surface of image-forming layer side ( $\mu_e$ )/coefficient of dynamic friction between material of smooth surface member of heat development apparatus and back surface ( $\mu_b$ )

In the present invention, the lubricity between the materials of the heat development apparatus and the surface of image-forming layer side and/or the opposite back surface can be controlled by adding a lubricant to the outermost layers and adjusting its addition amount.

It is preferred that undercoat layers containing a vinylidene chloride copolymer comprising 70 weight % or more of repetition units of vinylidene chloride monomers. Such a vinylidene chloride copolymer is disclosed in JP-A-64-20544, JP-A-1-180537, JP-A-1-209443, JP-A-1-285939,

JP-A-1-296243, JP-A-2-24649, JP-A-2-24648, JP-A-2-184844, JP-A-3-109545, JP-A-3-137637, JP-A-3-141346, JP-A-3-141347, JP-A-4-96055, U.S. Pat. No. 4,645,731, JP-A-4-68344, Japanese Patent No. 2,557,641, page 2, right column, line 20 to page3, right column, line 30, JP-A-2000-39684, paragraphs 0020–0037, and Japanese Patent Application No. 11-106881, paragraphs 0063–0080.

If the vinylidene chloride monomer content is less than 70 weight %, sufficient moisture resistance cannot be obtained, and dimensional change with time after the heat development will become significant. The vinylidene chloride copolymer preferably contains repetition units of carboxyl group-containing vinyl monomers, besides the repetition units of vinylidene chloride monomer. A polymer consists solely of vinylidene chloride monomers crystallizes, and

therefore it becomes difficult to form a uniform film when a moisture resistant layer is coated. Further, carboxyl group-containing vinyl monomers are indispensable for stabilizing the polymer. For these reasons, the repetition units of carboxyl group-containing vinyl monomers are added to the polymer.

The vinylidene chloride copolymer used in the present invention preferably has a molecular weight of 45,000 or

less, more preferably 10,000–45,000, as a weight average molecular weight. When the molecular weight becomes large, adhesion between the vinylidene chloride copolymer layer and the support layer composed of polyester or the like tends to be degraded.

The content of the vinylidene chloride copolymer used in the present invention is such an amount that the undercoat layers should have a thickness of 0.3  $\mu\text{m}$  or more, preferably 0.3  $\mu\text{m}$  to 4  $\mu\text{m}$ , as a total thickness of the undercoat layers containing the vinylidene chloride copolymer for one side.

The vinylidene chloride copolymer layer as an undercoat layer is preferably provided a first undercoat layer, which is directly coated on the support, and usually one vinylidene chloride copolymer layer is provided for each side. However, two or more of layers may be provided as the case may be. When multiple layers consisting of two or more layers are provided, the total amount of the vinylidene chloride copolymer may be within the range of the present invention defined above.

Such an undercoat layer may contain a crosslinking agent, matting agent or the like, in addition to the vinylidene chloride copolymer.

The support may be coated with an undercoat layer comprising SBR polyester, gelatin or the like as a binder, in addition to the vinylidene chloride copolymer layer, as required. These undercoat layers may have a multilayer structure, and may be provided on one side or both sides of the support. The undercoat layers generally have a thickness (per layer) of 0.01–5  $\mu\text{m}$ , more preferably 0.05–1  $\mu\text{m}$ .

For the photothermographic material of the present invention, various kinds of supports can be used. Typical supports comprise polyester such as polyethylene terephthalate, and polyethylene naphthalate, cellulose nitrate, cellulose ester, polyvinylacetal, syndiotactic polystyrene, polycarbonate, paper support of which both surfaces are coated with polyethylene or the like. Among these, biaxially stretched polyester, especially polyethylene terephthalate (PET), is preferred in view of strength, dimensional stability, chemical resistance and so forth. The support preferably has a thickness of 90–180  $\mu\text{m}$  as a base thickness except for the undercoat layers.

Preferably used as the support of the photothermographic material of the present invention is a polyester film, in particular polyethylene terephthalate film, subjected to a heat treatment in a temperature range of 130–185° C. in order to relax the internal distortion formed in the film during the biaxial stretching so that thermal shrinkage distortion occurring during the heat development could be eliminated. Such films are described in JP-A-10-48772, JP-A-10-10676, JP-A-10-10677, JP-A-11-65025 and JP-A-11-138648.

After such a heat treatment, the support preferably shows dimensional changes caused by heating at 120° C. for 30 seconds of –0.03% to +0.01% for the machine direction (MD) and 0 to 0.04% for the transverse direction (TD).

The photothermographic material of the present invention can be subjected to an antistatic treatment using the conductive metal oxides and/or fluorinated surfactants disclosed in JP-A-11-84573, paragraphs 0040–0051 for the purposes of reducing adhesion of dusts, preventing generation of static marks, preventing transportation failure during the automatic transportation and so forth. As the conductive metal oxides, the conductive acicular tin oxide doped with antimony disclosed in U.S. Pat. No. 5,575,957 and JP-A-11-223901, paragraphs 0012–0020 and the fibrous tin oxide doped with antimony disclosed in JP-A-4-29134 can be preferably used.

The layer containing a metal oxide should show a surface specific resistance (surface resistivity) of  $10^{12}$   $\Omega$  or less, preferably  $10^{11}$   $\Omega$  or less, in an atmosphere at 25° C. and 20% of relative humidity. Such a resistivity provides good 5 antistatic property. Although the surface resistivity is not particularly limited as for the lower limit, it is usually about  $10^7$   $\Omega$ .

The photothermographic material of the present invention preferably has a Beck's smoothness of 2000 seconds or less, 10 more preferably 10 seconds to 2000 seconds, as for at least one of the outermost surfaces of the image-forming layer side and the opposite side, preferably for the both sides.

Beck smoothness can be easily determined according to Japanese Industrial Standard (JIS) P8119, "Test Method for 15 Smoothness of Paper and Paperboard by Beck Test Device" and TAPPI Standard Method T479.

Beck smoothness of the outermost surfaces of the image-forming layer side and the opposite side of the photothermographic material can be controlled by suitably selecting 20 particle size and amount of matting agent to be contained in the layers constituting the surfaces as described in JP-A-11-84573, paragraphs 0052–0059.

In the present invention, water-soluble polymers are preferably used as a thickener for imparting coating property. 25 The polymers may be either naturally occurring polymers or synthetic polymers, and types thereof are not particularly limited. Specifically, there are mentioned naturally occurring polymers such as starches (corn starch, starch etc.), seaweeds (agar, sodium arginate etc.), vegetable adhesive substances (gum arabic etc.), animal proteins (glue, casein, gelatin, egg white etc.) and adhesive fermentation products (pullulan, dextrin etc.), semi-synthetic polymers such as semi-synthetic starches (soluble starch, carboxyl starch, dextran etc.) and semi-synthetic celluloses (viscose, 30 methylcellulose, ethylcellulose, carboxymethylcellulose, hydroxyethylcellulose, hydroxypropylcellulose, hydroxypropylmethylcellulose etc.), synthetic polymers (polyvinyl alcohol, polyacrylamide, polyvinylpyrrolidone, polyethylene glycol, polypropylene glycol, polyvinyl ether, polyethylene-imine, polystyrenesulfonic acid or styrenesulfonic acid copolymer, polyvinylsulfonic acid or vinylsulfonic acid copolymer, polyacrylic acid or acrylic acid copolymer, acrylic acid or acrylic acid copolymer, maleic acid copolymer, maleic acid monoester copolymer, 35 polyacryloyl methylpropanesulfonate or acryloyl methylpropanesulfonate copolymer) and so forth.

Among these, water-soluble polymers preferably used are sodium arginate, gelatin, dextrin, methylcellulose, carboxymethylcellulose, hydroxyethylcellulose, 40 hydroxypropylcellulose, polyvinyl alcohol, polyacrylamide, polyvinylpyrrolidone, polyethylene glycol, polypropylene glycol, polystyrenesulfonic acid or styrenesulfonic acid copolymer, polyacrylic acid or acrylic acid copolymer, maleic acid monoester copolymer, polyacryloylmethyl propanesulfonate or acryloylmethyl propanesulfonate copolymer, and they are particularly preferably used as a thickener.

Among these, particularly preferred thickeners are gelatin, dextrin, methylcellulose, carboxymethylcellulose, 45 hydroxyethylcellulose, polyvinyl alcohol, polyacrylamide, polyvinylpyrrolidone, polystyrenesulfonate or styrenesulfonate copolymer, polyacrylic acid or acrylic acid copolymer, maleic acid monoester copolymer and so forth. These compounds are described in detail in "Shin Suiyosei Polymer no Oyo to Shijo (Applications and Market of Water-soluble Polymers, New Edition)", CMC Shuppan, Inc., Ed. by Shinji Nagatomo, Nov. 4, 1988.

The amount of the water-soluble polymers used as a thickener is not particularly limited so long as viscosity is increased when they are added to a coating solution. Their concentration in the solution is generally 0.01 to 30 weight %, preferably 0.05 to 20 weight %, particularly preferably 0.1 to 10 weight %. Viscosity to be increased by the polymers is preferably 1-200 mPa·s, more preferably 5-100 mPa·s, as increased degree of viscosity compared with the initial viscosity. The viscosity is represented with values measured at 25° C. by using B type rotational viscometer. Upon addition to a coating solution or the like, it is generally desirable that the thickener is added as a solution diluted as far as possible. It is also desirable to perform the addition with sufficient stirring.

Surfactants used in the present invention will be described below. The surfactants used in the present invention are classified into dispersing agents, coating agents, wetting agents, antistatic agents, photographic property controlling agents and so forth depending on the purposes of use thereof, and the purposes can be attained by suitably selecting the surfactants described below and using them. As the surfactants used in the present invention, any of nonionic or ionic (anionic, cationic, betaine) surfactants can be used. Further, fluorinated surfactants can also be preferably used.

Preferred examples of the nonionic surfactant include surfactants having polyoxyethylene, polyoxypropylene, polyoxybutylene, polyglycidyl, sorbitan or the like as the nonionic hydrophilic group. Specifically, there can be mentioned polyoxyethylene alkyl ethers, polyoxyethylene alkyl phenyl ethers, polyoxyethylene/polyoxypropylene glycols, polyhydric alcohol aliphatic acid partial esters, polyoxyethylene polyhydric alcohol aliphatic acid partial esters, polyoxyethylene aliphatic acid esters, polyglycerin aliphatic acid esters, aliphatic acid diethanolamides, triethanolamine aliphatic acid partial esters and so forth.

Examples of anionic surfactants include carboxylic acid salts, sulfuric acid salts, sulfonic acid salts and phosphoric acid salts. Typical examples thereof are aliphatic acid salts, alkylbenzenesulfonates, alkylnaphthalenesulfonates, alkylsulfonates,  $\alpha$ -olefinsulfonates, dialkylsulfosuccinates,  $\alpha$ -sulfonated aliphatic acid salts, N-methyl-N-oleyltaurine, petroleum sulfonates, alkylsulfates, sulfated fats and oils, polyoxyethylene alkyl ether sulfates, polyoxyethylene alkyl phenyl ether sulfates, polyoxyethylene styrenylphenyl ether sulfates, alkyl phosphates, polyoxyethylene alkyl ether phosphates, naphthalenesulfonate formaldehyde condensates and so forth.

Examples of the cationic surfactants include amine salts, quaternary ammonium salts, pyridinium salts and so forth, and primary to tertiary amine salts and quaternary ammonium salts (tetraalkylammonium salts, trialkylbenzylammonium salts, alkylpyridinium salts, alkylimidazolium salts etc.) can be mentioned.

Examples of betaine type surfactants include carboxybetaine, sulfobetaine and so forth, and N-trialkyl-N-carboxymethylammonium betaine, N-trialkyl-N-sulfoalkylammonium betaine and so forth can be mentioned.

These surfactants are described in Takao Kariyone, "Kaimen Kasseizai no Oyo (Applications of Surfactants)", Sawai Shobo, Sep. 1, 1980). In the present invention, amounts of the preferred surfactants are not particularly limited, and they can be used in an amount providing desired surface activating property. The coating amount of the fluorine-containing surfactants is preferably 0.01-250 mg per 1 m<sup>2</sup>.

Specific examples of the surfactants are mentioned below. However, the surfactants are not limited to these (—C<sub>6</sub>H<sub>4</sub>— represents phenylene group in the following formulas).

- WA-1: C<sub>16</sub>H<sub>33</sub>(OCH<sub>2</sub>CH<sub>2</sub>)<sub>10</sub>OH
- WA-2: C<sub>9</sub>H<sub>19</sub>—C<sub>6</sub>H<sub>4</sub>—(OCH<sub>2</sub>CH<sub>2</sub>)<sub>12</sub>OH
- WA-3: Sodium dodecylbenzenesulfonate
- WA-4: Sodium tri(isopropyl)naphthalenesulfonate
- WA-5: Sodium tri(isobutyl)naphthalenesulfonate
- WA-6: Sodium dodecylsulfate
- WA-7:  $\alpha$ -Sulfasuccinic acid di(2-ethylhexyl) ester sodium salt
- WA-8: C<sub>8</sub>H<sub>17</sub>—C<sub>6</sub>H<sub>4</sub>—(CH<sub>2</sub>CH<sub>2</sub>O)<sub>3</sub>(CH<sub>2</sub>)<sub>2</sub>SO<sub>3</sub>K
- WA-10: Cetyltrimethylammonium chloride
- WA-11: C<sub>11</sub>H<sub>23</sub>CONHCH<sub>2</sub>CH<sub>2</sub>N<sup>(+)</sup>(CH<sub>3</sub>)<sub>2</sub>—CH<sub>2</sub>COO<sup>(-)</sup>
- WA-12: C<sub>8</sub>F<sub>17</sub>SO<sub>2</sub>N(C<sub>3</sub>H<sub>7</sub>)(CH<sub>2</sub>CH<sub>2</sub>O)<sub>16</sub>H
- WA-13: C<sub>8</sub>F<sub>17</sub>SO<sub>2</sub>N(C<sub>3</sub>H<sub>7</sub>)CH<sub>2</sub>COOK
- WA-14: C<sub>8</sub>F<sub>17</sub>SO<sub>3</sub>K
- WA-15: C<sub>8</sub>F<sub>17</sub>SO<sub>2</sub>N(C<sub>3</sub>H<sub>7</sub>)(CH<sub>2</sub>CH<sub>2</sub>O)<sub>4</sub>(CH<sub>2</sub>)<sub>4</sub>SO<sub>3</sub>Na
- WA-16: C<sub>8</sub>F<sub>17</sub>SO<sub>2</sub>N(C<sub>3</sub>H<sub>7</sub>)(CH<sub>2</sub>)<sub>3</sub>OCH<sub>2</sub>CH<sub>2</sub>N<sup>(+)</sup>(CH<sub>3</sub>)<sub>3</sub>—CH<sub>3</sub>·C<sub>6</sub>H<sub>4</sub>—SO<sub>3</sub><sup>(-)</sup>
- WA-17: C<sub>8</sub>F<sub>17</sub>SO<sub>2</sub>N(C<sub>3</sub>H<sub>7</sub>)CH<sub>2</sub>CH<sub>2</sub>CH<sub>2</sub>N<sup>(+)</sup>(CH<sub>3</sub>)<sub>2</sub>—CH<sub>2</sub>COO<sup>(-)</sup>

20 In a preferred embodiment of the present invention, an intermediate layer may be provided as required in addition to the image-forming layer and the protective layer. To improve the productivity or the like, it is preferred that these multiple layers should be simultaneously coated as stacked layers by using aqueous systems. While extrusion coating, slide bead coating, curtain coating and so forth can be mentioned as the coating method, the slide bead coating method shown in JP-A-2000-2964, FIG. 1 is particularly preferred.

30 Silver halide photographic photosensitive materials utilizing gelatin as a main binder are rapidly cooled in a first drying zone, which is provided downstream from a coating dye. As a result, the gelatin gels and the coated film is solidified by cooling. The coated film that no longer flows as 35 a result of the solidification by cooling is transferred to a second drying zone, and the solvent in the coating solution is evaporated in this drying zone and subsequent drying zones so that a film is formed. As drying method after the second drying zone, there can be mentioned the air loop 40 method where a support supported by rollers is blown by air jet from a U-shaped duct, the helix method (air floating method) where the support is helically wound around a cylindrical duct and dried during transportation and so forth.

When the layers are formed by using coating solutions 45 comprising polymer latex as a main component of binder, the flow of the coating solution cannot be stopped by rapid cooling. Therefore, the predrying may be insufficient only with the first drying zone. In such a case, if such a drying method as utilized for silver halide photographic photosensitive materials is used, uneven flow or uneven drying may 50 occur, and therefore serious defects are likely to occur on the coated surface.

The preferred drying method for the present invention is such a method as described in JP-A-2000-2964, where the drying is attained in a horizontal drying zone irrespective of the drying zone, i.e., the first or second drying zone, at least until the constant rate drying is finished. The transportation 55 of the support during the period immediately after the coating and before the support is introduced into the horizontal drying zone may be performed either horizontally or not horizontally, and the rising angle of the material with respect to the horizontal direction of the coating machine 60 may be within the range of 0-70°. Further, in the horizontal drying zone used in the present invention, the support may be transported at an angle within  $\pm 15^\circ$  with respect to the horizontal direction of the coating machine, and it does not 65 mean exactly horizontal transportation.

The constant rate drying used in the present invention means a drying process in which all entering calorie is consumed for evaporation of solvent at a constant liquid film temperature. Decreasing rate drying means a drying process where the drying rate is reduced by various factors (for example, diffusion of moisture in the material for transfer becomes a rate-limiting factor, evaporation surface is recessed etc.) in an end period of the drying, and imparted calorie is also used for increase of liquid film temperature. The critical moisture content for the transition from the constant rate drying to the decreasing rate drying is 200–300%. When the constant rate drying is finished, the drying has sufficiently progressed so that the flowing could be stopped, and therefore such a drying method as used for silver halide photographic photosensitive materials may also be employable. In the present invention, however, it is preferred that the drying should be performed in a horizontal drying zone until the final drying degree is attained even after the constant rate drying.

As for the drying condition for forming the image-forming layer and/or protective layer, it is preferred that the liquid film surface temperature during the constant rate drying should be higher than minimum film forming temperature (MTF) of polymer latex (MTF is usually higher than glass transition temperature  $T_g$  of polymer by 3–5°C.). In many cases, it is usually selected from the range of 25–40°C., because of limitations imposed by production facilities. Further, the dry bulb temperature during the decreasing rate drying is preferably lower than  $T_g$  of the support (in the case of PET, usually 80°C. or lower). The liquid film surface temperature referred to in this specification means a solvent liquid film surface temperature of coated liquid film coated on a support, and the dry bulb temperature means a temperature of drying air blow in the drying zone.

If the constant rate drying is performed under a condition that lowers the liquid film surface temperature, the drying is likely to become insufficient. Therefore, the film-forming property of the protective layer is markedly degraded, and it becomes likely that cracks will be generated on the film surface. Further, film strength also becomes weak and thus it becomes likely that there arise serious problems, for example, the film becomes liable to suffer from scratches during transportation in a light exposure apparatus or heat development apparatus.

On the other hand, if the drying is performed under a condition that elevates the liquid film surface temperature, the protective layer mainly consisting of polymer latex rapidly becomes a film, but the under layers including the image-forming layer do not lose flowability, and hence it is likely that unevenness is formed on the surface. Furthermore, if the support (base) is subjected to a temperature higher than its  $T_g$ , dimensional stability and resistance to curl tendency tends to be degraded.

While the same is applied to the serial coating, in which an under layer is coated and then an upper layer is coated, as for properties of coating solutions, when an upper layer and a lower layer are coated as stacked layers by coating the upper layer before drying of the lower layer, in particular, a coating solution for the image-forming layer and a coating solution for protective layer preferably show a pH difference of 2.5 or less, and a smaller value of this pH difference is more preferred. If the pH difference becomes large, it becomes likely that microscopic aggregations are generated at the interface of the coating solutions and thus it becomes likely that serious defects of surface condition such as coating stripes occur during continuous coating for a long length.

The coating solution for the image-forming layer preferably has a viscosity of 15–100 mPa·S, more preferably 30–70 mPa·S, at 25°C. The coating solution for the protective layer preferably has a viscosity of 5–75 mPa·S, more preferably 20–50 mPa·S, at 25°C. These viscosities are measured by using a B-type viscometer.

The rolling up after the drying is preferably carried out under conditions of a temperature of 20–30°C. and a relative humidity of 45±20%. As for rolled shape, the material may be rolled so that the surface of the image-forming layer side may be toward the outside or inside of the roll according to a shape suitable for subsequent processing. Further, it is also preferred that, when the material is further processed in a rolled shape, the material should be rolled up into a shape of roll in which the sides are reversed compared with the original rolled shape during processing, in order to eliminate the curl generated while the material is in the original rolled shape. Relative humidity of the photosensitive material is preferably controlled to be in the range of 20–55% (measured at 25°C.).

In conventional coating solutions for photographic emulsions, which are viscous solutions containing silver halide and gelatin as a base, air bubbles are dissolved in the solutions and eliminated only by feeding the solution by pressurization, and air bubbles are scarcely formed even when the solutions are placed under atmospheric pressure again for coating. However, as for the coating solution for the image-forming layer containing dispersion of silver salt of organic acid, polymer latex and so forth preferably used in the present invention, only feeding of it by pressurization is likely to result in insufficient degassing. Therefore, it is preferably fed so that air/liquid interfaces could not be produced, while giving ultrasonic vibration to perform degassing.

In the present invention, the degassing of a coating solution is preferably performed by a method where the coating solution is degassed under reduced pressure before coating, and further the solution is maintained in a pressurized state at a pressure of 1.5 kg/cm<sup>2</sup> and continuously fed so that air/liquid interfaces could not be formed, while giving ultrasonic vibration to the solution. Specifically, the method disclosed in JP-B-55-6405 (from page 4, line 20 to page 7, line 11) is preferred. As an apparatus for performing such degassing, the apparatus disclosed in Japanese Patent Application No. 10-290003, examples and FIG. 3, is preferably used.

The pressurization condition is preferably 1.5 kg/cm<sup>2</sup> or more, more preferably 1.8 kg/cm<sup>2</sup> or more. While the pressure is not particularly limited as for its upper limit, it is usually about 5 kg/cm<sup>2</sup> or less. Ultrasonic wave given to the solution should have a sound pressure of 0.2 V or more, preferably 0.5 V to 3.0 V. Although a higher sound pressure is generally preferred, an unduly high sound pressure provides high temperature portions due to cavitation, which may causes fogging. While frequency of the ultrasonic wave is not particularly limited, it is usually 10 kHz or higher, preferably 20 kHz to 200 kHz. The degassing under reduced pressure means a process where a coating solution is placed in a sealed tank (usually a tank in which the solution is prepared or stored) under reduced pressure to increase diameters of air bubbles in the coating solution so that degassing could be attained by buoyancy imparted to the air bubbles. The reduced pressure condition for the degassing under reduced pressure is –200 mmHg or a pressure condition lower than that, preferably –250 mmHg or a pressure condition lower than that. Although the lower limit of the pressure condition is not particularly limited, it is usually

about -800 mmHg or higher. Time under the reduced pressure is 30 minutes or more, preferably 45 minutes or more, and its upper limit is not particularly limited.

In the present invention, the image-forming layer, protective layer for the image-forming layer, undercoat layer and back layer may contain a dye in order to prevent halation and so forth as disclosed in JP-A-11-84573, paragraphs 0204-0208 and Japanese Patent Application No. 11-106881, paragraphs 0240-0241.

Various dyes and pigments can be used for the image-forming layer for improvement of color tone and prevention of irradiation. While arbitrary dyes and pigments may be used for the image-forming layer, the compounds disclosed in JP-A-11-119374, paragraphs 0297, for example, can be used. These dyes may be added in any form such as solution, emulsion, solid microparticle dispersion and macromolecule mordant mordanted with the dyes. Although the amount of these compounds is determined by the desired absorption, they are preferably used in an amount of  $1 \times 10^{-6}$  g to 1 g per 1 m<sup>2</sup>, in general.

When an antihalation dye is used in the present invention, the dye may be any compound so long as it shows intended absorption in a desired range and sufficiently low absorption in the visible region after development, and provides a preferred absorption spectrum pattern of the back layer. For example, the compounds disclosed in JP-A-11-119374, paragraph 0300 can be used. There can also be used a method of reducing density obtained with a dye by thermal decoloration as disclosed in Belgian Patent No. 733,706, a method of reducing the density by decoloration utilizing light irradiation as disclosed in JP-A-54-17833 and so forth.

When the photothermographic material of the present invention after heat development is used as a mask for the production of printing plate from a PS plate, the photothermographic material after heat development carries information for setting up light exposure conditions of platemaking machine for PS plates or information for setting up platemaking conditions including transportation conditions of mask originals and PS plates as image information. Therefore, in order to read such information, densities (amounts) of the aforementioned irradiation dye, halation dye and filter dye are limited. Because the information is read by LED or laser, Dmin (minimum density) in a wavelength region of the sensor must be low, i.e., the absorbance must be 0.3 or less. For example, a platemaking machine S-FNRIII produced by Fuji Photo Film Co., Ltd. uses a light source having a wavelength of 670 nm for a detector for detecting resister marks and a bar code reader. Further, platemaking machines of APML series produced by Shimizu Seisaku Co., Ltd. utilize a light source at 670 nm as a bar code reader. That is, if Dmin (minimum density) around 670 nm is high, the information on the film cannot be correctly detected, and thus operation errors such as transportation failure, light exposure failure and so forth are caused in platemaking machines. Therefore, in order to read information with a light source of 670 nm, Dmin around 670 nm must be low and the absorbance at 660-680 nm after the heat development must be 0.3 or less, more preferably 0.25 or less. Although the absorbance is not particularly limited as for its lower limit, it is usually about 0.10.

In the present invention, as the exposure apparatus used for the imagewise light exposure, any apparatus may be used so long as it is an exposure apparatus enabling light exposure with an exposure time of  $10^{-7}$  second or shorter. However, a light exposure apparatus utilizing a laser diode (LD) or a light emitting diode (LED) as a light source is preferably used in general. In particular, LD is more preferred in view

of high output and high resolution. Any of these light sources may be used so long as they can emit a light of electromagnetic wave spectrum of desired wavelength range. For example, as for LD, dye lasers, gas lasers, solid state lasers, semiconductor lasers and so forth can be used.

The light exposure in the present invention is performed with overlapped light beams of light sources. The term "overlapped" means that a vertical scanning pitch width is smaller than the diameter of the beams. For example, the overlap can be quantitatively expressed as FWHM/vertical-scanning pitch width (overlap coefficient), where the beam diameter is represented as a half width of beam strength (FWHM). In the present invention, it is preferred that this overlap coefficient is 0.2 or more. Laser energy density on the surface of the photothermographic material surface is preferably several to several hundreds of microjoules ( $\mu$ J) per cm<sup>2</sup>, more preferably several to several tens of microjoules per cm<sup>2</sup>.

The scanning method of the light source of the light exposure apparatus used in the present invention is not particularly limited, and the cylinder external surface scanning method, cylinder internal surface scanning method, flat surface scanning method and so forth can be used. Although the channel of light source may be either single channel or multichannel, a multichannel comprising two or more of laser heads is preferred, because it provides high output and shortens writing time. In particular, for the cylinder external surface scanning method, a multichannel carrying several to several tens of laser heads is preferably used.

The photothermographic material of the present invention shows low haze upon the light exposure, and therefore it is likely to generate interference fringes. As techniques for preventing such interference fringes, there are known a technique of obliquely irradiating a photosensitive material with a laser light as disclosed in JP-A-5-113548, a technique of utilizing a multimode laser disclosed in WO95/31754 and so forth, and these techniques are preferably used.

Although any method may be used for the heat development process of the image-forming method used for the present invention, the development is usually performed by heating a photothermographic material exposed imagewise. As preferred embodiments of heat development apparatus to be used, there are heat development apparatuses in which a photothermographic material is brought into contact with a heat source such as heat roller or heat drum as disclosed in JP-B-5-56499, JP-A-9-292695, JP-A-9-297385 and WO95/30934, and heat development apparatuses of non-contact type as disclosed in JP-A-7-13294, WO97/28489, WO97/28488 and WO97/28487. Particularly preferred embodiments are the heat development apparatuses of non-contact type. The temperature for the development is preferably 80° C. to 250° C., more preferably 100° C. to 140° C. The development time is preferably 1 to 180 seconds, more preferably 5 to 90 seconds. The line speed is preferably 140 cm/minute or more, more preferably 150 cm/minute or more.

As a method for preventing uneven development due to dimensional change of the photothermographic material during the heat development, it is effective to employ a method for forming images wherein the material is heated at a temperature of 80° C. or higher but lower than 115° C. for 5 seconds or more so as not to develop images, and then subjected to heat development at 110-140° C. to form images (so-called multi-step heating method).

Since the photothermographic material of the present invention is subjected to a high temperature of 110° C. or higher during the heat development, a part of the compo-

nents contained in the material or a part of decomposition products produced by the heat development are volatilized. It is known that these volatilized components exert various bad influences, for example, they may cause uneven development, erode structural members of development apparatuses, deposit at low temperature portions as dusts to cause deformation of image surface, adhere to image surface as stains and so forth. As a method for eliminating these influences, it is known to provide a filter on the heat development apparatus, or suitably control air flows in the heat development apparatus. These methods may be effectively used in combination.

WO95/30933, WO97/21150 and International Patent Publication in Japanese (Kohyo) No. 10-500496 disclose use of a filter cartridge containing binding absorption particles and having a first vent for introducing volatilized components and a second vent for discharging them in heating means for heating a photothermographic material by contact. Further, WO96/12213 and International Patent Publication in Japanese (Kohyo) No. 10-507403 disclose use of a filter consisting of a combination of heat conductive condensation collector and a gas-absorptive microparticle filter. These can be preferably used in the present invention.

Further, U.S. Pat. No. 4,518,845 and JP-B-3-54331 disclose structures comprising means for eliminating vapor from a photothermographic material, pressing means for pressing a photothermographic material to a heat-conductive member and means for heating the heat-conductive member. Further, WO98/27458 discloses elimination of components volatilized from a photothermographic material and increasing fog from a surface of the photothermographic material. These techniques are also preferably used for the present invention.

An example of the structure of heat development apparatus used for the heat development of the photothermographic material of the present invention is shown in FIG. 1. FIG. 1 depicts a side view of a heat development apparatus. The heat development apparatus shown in FIG. 1 comprises carrying-in roller pairs 11 (upper rollers are silicone rubber rollers, and lower rollers are aluminum heating rollers), which carry a photothermographic material 10 into the heating section while making the material in a flat shape and preheating it, and carrying-out roller pairs 12, which carry out the photothermographic material 10 after heat development from the heating section while maintaining the material to be in a flat shape. The photothermographic material 10 is heat-developed while it is conveyed by the carrying-in roller pairs 11 and then by the carrying-out roller pairs 12. A conveying means for carrying the photothermographic material 10 under the heat development is provided with multiple rollers 13 so that they could be contacted with the surface of the image-forming layer side, and a flat surface 14 adhered with non-woven fabric (composed of, for example, aromatic polyamide, Teflon etc.) or the like is provided on the opposite side so that it could be contacted with the back surface. The photothermographic material 10 is conveyed by driving of the multiple rollers 13 contacted with the image-forming layer side, while the back surface slides on the flat surface 14. Heaters 15 are provided over the rollers 13 and under the flat surface 14 so that the photothermographic material 10 could be heated from the both sides. Examples of the heating means include panel heaters and so forth. While clearance between the rollers 13 and the flat surface 14 may vary depending on the material of the flat surface member, it is suitably adjusted to a clearance that allows the conveyance of the photothermographic material 10. The clearance is preferably 0-1 mm.

The materials of the surfaces of the rollers 13 and the member of the flat surface 14 may be composed of any materials so long as they have heat resistance and they should not cause any troubles in the conveyance of the photothermographic material 10. However, the material of the roller surface is preferably composed of silicone rubber, and the member of the flat surface is preferably composed of non-woven fabric made of aromatic polyamide or Teflon (PTFE). The heating means preferably comprises multiple heaters so that temperature of each heater can be adjusted freely.

The heating section is constituted by a preheating section A comprising the carrying-in roller pairs 11 and a heat development section B comprising the heaters 15. Temperature of the preheating section A locating upstream from the heat development section B is preferably controlled to be lower than the heat development temperature (for example, lower by about 10-30° C.), and temperature and heat development time are desirably adjusted so that they could be sufficient for evaporating moisture contained in the photothermographic material 10. The temperature is also adjusted to be higher than the glass transition temperature (Tg) of the support of the photothermographic material 10 so that uneven development could be prevented. Temperature distribution of the preheating section and the heat development section is preferably  $\pm 1^\circ$  C. or less, more preferably  $\pm 0.5^\circ$  C. or less.

Moreover, guide panels 16 are provided downstream from the heat development section B, and they constitute a gradual cooling section C together with the carrying-out roller pairs 12.

The guide panels 16 are preferably composed of a material of low heat conductivity, and it is preferred that the cooling is performed gradually so as not to cause deformation of the photothermographic material 10. The cooling rate is preferably 0.5-10° C./second.

The heat development apparatus was explained with reference to the example shown in the drawing. However, the apparatus is not limited to the example. For example, the heat development apparatus used for the present invention may have a variety of structures such as one disclosed in JP-A-7-13294. For the multi-stage heating method, which is preferably used for the present invention, the photothermographic material may be successively heated at different temperatures in such an apparatus as mentioned above, which is provided with two or more heat sources at different temperatures.

## EXAMPLES

The present invention will be specifically explained with reference to the following examples. The materials, regents, ratios, procedures and so forth shown in the following examples can be optionally changed so long as such change does not depart from the spirit of the present invention. Therefore, the scope of the present invention is not limited by the following examples.

### <Example 1

#### Preparation of Silver Halide Emulsion A

In 700 ml of water, 11 g of alkali-treated gelatin (calcium content: 2700 ppm or less), 30 mg of potassium bromide and 1.3 g of sodium 4-methylbenzenesulfonate were dissolved. After the solution was adjusted to pH 6.5 at a temperature of 40° C., 159 ml of an aqueous solution containing 18.6 g of silver nitrate and an aqueous solution containing 1 mol/l of potassium bromide,  $5 \times 10^{-6}$  mol/l of  $(\text{NH}_4)_2\text{RhCl}_5(\text{H}_2\text{O})$  and

31

$2 \times 10^{-5}$  mol/l of  $K_3IrCl_6$  were added by the control double jet method over 6 minutes and 30 seconds while pAg was maintained at 7.7. Then, 476 ml of an aqueous solution containing 55.5 g of silver nitrate and an aqueous solution containing 1 mol/l of potassium bromide and  $2 \times 10^{-5}$  mol/l of  $K_3IrCl_6$  were added by the control double jet method over 28 minutes and 30 seconds while pAg was maintained at 7.7. Then, the pH was lowered to cause coagulation precipitation to effect desalting, 51.1 g of low molecular weight gelatin having an average molecular weight of 15,000 (calcium content: 20 ppm or less) was added, and pH and pAg were adjusted to 5.9 and 8.0, respectively. The grains obtained were cubic grains having a mean grain size of  $0.08 \mu\text{m}$ , variation coefficient of 9% for projected area and a [100] face ratio of 90%.

The temperature of the silver halide grains obtained as described above was raised to  $60^\circ\text{C}$ ., and the grains were added with  $76 \mu\text{mol}$  per mole of silver of sodium benzenethiobenzoate. After 3 minutes,  $71 \mu\text{mol}$  of triethylthiourea was further added, and the grains were ripened for 100 minutes, then added with  $5 \times 10^{-4}$  mol/l of 4-hydroxy-6-methyl-1,3,3a,7-tetraazaindene and 0.17 g of Compound A, and cooled to  $40^\circ\text{C}$ .

Then, while the mixture was maintained at  $40^\circ\text{C}$ ., it was added with potassium bromide (added as aqueous solution), the following Sensitizing Dye A (added as solution in ethanol) and Compound B (added as solution in methanol) were added in amounts of  $4.7 \times 10^{-2}$  mole,  $12.8 \times 10^{-4}$  mole and  $6.4 \times 10^{-3}$  mole per mole of the silver halide with stirring. After 20 minutes, the emulsion was quenched to  $30^\circ\text{C}$ . to complete the preparation of Silver halide emulsion A.

32

C. A mixture of 635 ml of distilled water and 30 ml of tert-butanol contained in a reaction vessel kept at  $30^\circ\text{C}$ . was added with the whole amount of the aforementioned sodium behenate solution and the whole amount of the aqueous silver nitrate solution with stirring at constant flow rates over the periods of 62 minutes and 10 seconds, and 60 minutes, respectively. In this operation, the aqueous silver nitrate solution was added in such a manner that only the aqueous silver nitrate solution should be added for 7 minutes and 20 seconds after starting the addition of the aqueous silver nitrate solution, and then the addition of the aqueous solution of sodium behenate was started and added in such a manner that only the aqueous solution of sodium behenate should be added for 9 minutes and 30 seconds after finishing the addition of the aqueous silver nitrate solution. During the addition, the outside temperature was controlled so that the temperature in the reaction vessel could be  $30^\circ\text{C}$ . and the liquid temperature should not be raised. The piping of the addition system for the sodium behenate solution was warmed by steam trace and the steam opening was controlled such that the liquid temperature at the outlet orifice of the addition nozzle should be  $75^\circ\text{C}$ . The piping of the addition system for the aqueous silver nitrate solution was maintained by circulating cold water outside a double pipe. The addition position of the sodium behenate solution and the addition position of the aqueous silver nitrate solution were arranged symmetrically with respect to the stirring axis as the center, and the positions were controlled to be at heights for not contacting with the reaction mixture.

After finishing the addition of the sodium behenate solution, the mixture was left with stirring for 20 minutes at the same temperature and then the temperature was



#### Preparation of Silver Behenate Dispersion A

In an amount of 87.6 g of behenic acid (Edenor C22-85R, trade name, produced by Henkel Co.), 423 ml of distilled water, 49.2 ml of 5 N aqueous solution of NaOH and 120 ml of tert-butanol were mixed and allowed to react with stirring at  $75^\circ\text{C}$ . for one hour to obtain a solution of sodium behenate. Separately, 206.2 ml of an aqueous solution containing 40.4 g of silver nitrate was prepared and kept at  $10^\circ\text{C}$ .

decreased to  $25^\circ\text{C}$ . Thereafter, the solid content was recovered by suction filtration and the solid content was washed with water until electric conductivity of the filtrate became  $30 \mu\text{S}/\text{cm}$ . The solid content obtained as described above was stored as a wet cake without being dried.

When the shape of the obtained silver behenate grains was evaluated by an electron microscopic photography, the grains were scaly crystals having a mean diameter of pro-

jected areas of  $0.52 \mu\text{m}$ , mean thickness of  $0.14 \mu\text{m}$  and variation coefficient of 15% for mean diameter as spheres.

Then, dispersion of silver behenate was prepared as follows. To the wet cake corresponding to 100 g of the dry solid content was added with 7.4 g of polyvinyl alcohol (PVA-217, trade name, average polymerization degree: about 1700) and water to make the total amount 385 g, and the mixture was pre-dispersed by a homomixer. Then, the pre-dispersed stock dispersion was treated three times by using a dispersing machine (Microfluidizer-M-110S-EH; trade name, produced by Microfluidex International Corporation, using G10Z interaction chamber) with a pressure controlled to be  $1750 \text{ kg/cm}^2$  to obtain Silver behenate dispersion A. During the cooling operation, a desired dispersion temperature was achieved by providing coiled heat exchangers fixed before and after the interaction chamber and controlling the temperature of the refrigerant.

The silver behenate grains contained in Silver behenate dispersion A obtained as described above were grains having a volume weight mean diameter of  $0.52 \mu\text{m}$  and variation coefficient of 15%. The measurement of the grain size was carried out by using Master Sizer X produced by Malvern Instruments Ltd. When the grains were evaluated by an electron microscopic photography, the ratio of the long side to the short side was 1.5, the grain thickness was  $0.14 \mu\text{m}$ , and a mean aspect ratio (ratio of diameter as sphere of projected area of grain and grain thickness) was 5.1.

**Preparation of Solid Microparticle Dispersion of Reducing Agent: 1,1-bis(2-hydroxy-3,5-dimethylphenyl)-3,5,5-trimethylhexane**

In an amount of 10 kg of 1,1-bis(2-hydroxy-3,5-dimethylphenyl)-3,5,5-trimethylhexane and 10 kg of 20 weight % aqueous solution of denatured polyvinyl alcohol (Poval MP203, produced by Kuraray Co. Ltd.) were added with 400 g of Safinol 104E (Nissin Kagaku Co.), 640 g of methanol and 16 kg of water, and mixed sufficiently to form slurry. The slurry was fed by a diaphragm pump to a sand mill of horizontal type (UVM-2, produced by Imex Co.) containing zirconia beads having a mean diameter of  $0.5 \text{ mm}$ , and dispersed for 3 hours and 30 minutes. Then, the slurry was added with 4 g of benzothiazolinone sodium salt and water so that the concentration of the reducing agent could become 25 weight % to obtain a solid microparticile dispersion of reducing agent. The reducing agent particles contained in the reducing agent dispersion obtained as described above had a median diameter of  $0.44 \mu\text{m}$ , maximum particle diameter of  $2.0 \mu\text{m}$  or shorter and variation coefficient of 19% for mean particle diameter. The obtained reducing agent dispersion was filtered through a polypropylene filter having a pore size of  $3.0 \mu\text{m}$  to remove dusts and so forth, and stored.

**Preparation of Solid Microparticle Dispersion of Organic Polyhalogenated Compound A**

In an amount of 10 kg of Organic polyhalogenated compound A: tribromomethyl(4-(2,4,6-trimethylphenylsulfonyl)phenyl)-sulfone, 10 kg of 20 weight % aqueous solution of denatured polyvinyl alcohol (Poval MP203, produced by Kuraray Co. Ltd.), 639 g of 20 weight % aqueous solution of sodium triisopropylnaphthalenesulfonate, 400 g of Safinol 104E (Nissin Kagaku Co.), 640 g of methanol and 16 kg of water were mixed sufficiently to form slurry. The slurry was fed by a diaphragm pump to a sand mill of horizontal type (UVM-2, produced by Imex Co.) containing zirconia beads having

a mean diameter of  $0.5 \text{ mm}$ , and dispersed for 5 hours. Then, the slurry was added with water so that the concentration of Organic polyhalogenated compound A could become 25 weight % to obtain solid microparticle dispersion of Organic polyhalogenated compound A. The particles of Organic polyhalogenated compound A contained in the dispersion obtained as described above had a median diameter of  $0.36 \mu\text{m}$ , maximum particle diameter of  $2.0 \mu\text{m}$  or shorter and variation coefficient of 18% for mean particle diameter. The obtained dispersion was filtered through a polypropylene filter having a pore size of  $3.0 \mu\text{m}$  to remove dusts and so forth, and stored.

**Preparation of Solid Microparticle Dispersion of Organic Polyhalogenated Compound B**

15 In an amount of 5 kg of Organic polyhalogenated compound B: tribromomethylnaphthylsulfone, 2.5 kg of 20 weight % aqueous solution of denatured polyvinyl alcohol (Poval MP203, produced by Kuraray Co. Ltd.), 213 g of 20 weight % aqueous solution of sodium triisopropylnaphthalenesulfonate and 10 kg of water were mixed sufficiently to a  
20 form slurry. The slurry was fed by a diaphragm pump to a sand mill of horizontal type (UVM-2, produced by Imex Co.) containing zirconia beads having a mean diameter of  $0.5 \text{ mm}$ , and dispersed for 5 hours. Then, the slurry was  
25 added with 2.5 g of benzothiazolinone sodium salt and water so that the concentration of Organic polyhalogenated compound B could become 20 weight % to obtain solid microparticle dispersion of Organic polyhalogenated compound B. The particles of the organic polyhalogenated compound  
30 contained in the dispersion obtained as described above had a median diameter of  $0.38 \mu\text{m}$ , maximum particle diameter of  $2.0 \mu\text{m}$  or shorter and variation coefficient of 20% for mean particle diameter. The obtained dispersion was filtered through a polypropylene filter having a pore size of  $3.0 \mu\text{m}$   
35 to remove dusts and so forth, and stored.

**Preparation of Aqueous Solution of Organic Polyhalogenated Compound C**

Preparation composition (amounts in 100 g of completed solution) and preparation method

|     |                                                                                           |         |
|-----|-------------------------------------------------------------------------------------------|---------|
| (1) | Water                                                                                     | 75.0 ml |
| (2) | 20 weight % Aqueous solution of sodium triisopropylnaphthalenesulfonate                   | 8.6 ml  |
| (3) | 5 weight % Aqueous solution of sodium dihydrogenorthophosphate dihydrate                  | 6.8 ml  |
| (4) | 1 mol/l aqueous solution of potassium hydroxide                                           | 9.5 ml  |
| (5) | Organic polyhalogenated compound C<br>(3-tribromomethanesulfonylbenzoyl-aminoacetic acid) | 4.0 g   |

55 A solution was prepared as follows.

1. (1) to (4) were successively added at room temperature with stirring, and the mixture was stirred for 5 minutes after the addition of (4).
2. Further, the mixture was added with powder of (5), and it was dissolved until the solution became transparent.
3. The obtained aqueous solution was filtered through a polyester screen of 200 mesh to remove dusts and so forth, and stored.

**Preparation of Emulsion Dispersion of Compound Z**

In an amount of 10 kg of R-054 (Sanko Co., Ltd.) containing 85 weight % of Compound Z was mixed with

11.66 kg of MIBK and dissolved in the solvent at 80° C. for 1 hour in an atmosphere substituted with nitrogen. This solution was added with 25.52 kg of water, 12.76 kg of 20 weight % aqueous solution of MP polymer (MP-203, produced by Kuraray Co., Ltd.) and 0.44 kg of 20 weight % aqueous solution of sodium triisopropylnaphthalene-sulfonate and subjected to emulsion dispersion at 20–40° C. and 3600 rpm for 60 minutes. The dispersion was added with 0.08 kg of Safinol 104E (Nisshin Kagaku Co.) and 47.94 kg of water and distilled under reduced pressure to remove MIBK. Then, the concentration of Compound Z was adjusted to 10 weight %. The particles of Compound Z contained in the dispersion obtained as described above had a median diameter of 0.19  $\mu\text{m}$ , maximum particle diameter of 1.5  $\mu\text{m}$  or shorter and variation coefficient of 17% for mean particle diameter. The obtained dispersion was filtered through a polypropylene filter having a pore size of 3.0  $\mu\text{m}$  to remove dusts and so forth, and stored.

Preparation of Dispersion of 6-isopropylphthalazine  
Compound

Preparation composition (amounts in 100 g of completed dispersion) and preparation method

|     |                                                                                                  |         |
|-----|--------------------------------------------------------------------------------------------------|---------|
| (1) | Water                                                                                            | 86.15 g |
| (2) | Denatured polyvinyl alcohol<br>(Poval MP203, produced by Kuraray Co., Ltd.)                      | 2.0 g   |
| (3) | 10 weight % aqueous solution<br>of polyvinyl alcohol<br>(PVA-217, produced by Kuraray Co., Ltd.) | 7.0 g   |
| (4) | 20 weight % aqueous solution<br>of sodium triisopropylnaphthalene-sulfonate                      | 3.0 g   |
| (5) | 6-Isopropylphthalazine<br>(70% aqueous solution)                                                 | 7.15 g  |

Dispersion was prepared as follows.

- (1) was added with (2) at room temperature with stirring so that (2) could not coagulate, and mixed by stirring for 10 minutes.
- Then, the mixture was heated until the internal temperature reached 50° C., and stirred for 90 minutes to attain uniform dissolution.
- The internal temperature was lowered to 40° C. or lower, and the mixture was added with (3), (4) and (5) and stirred for 30 minutes to obtain a transparent dispersion.
- The obtained dispersion was filtered through a polypropylene filter having a pore size of 3.0  $\mu\text{m}$  to remove dusts and so forth, and stored.

Preparation of Solid Microparticle Dispersion of  
Nucleating Agent Y

In an amount of 4 kg of Nucleating agent Y, 1 kg of Poval PVA-217 (produced by Kuraray Co., Ltd.) and 36 kg of water were mixed sufficiently to form slurry. The slurry was fed by a diaphragm pump to a sand mill of horizontal type (UVM-2, produced by Imex Co.) containing zirconia beads having a mean diameter of 0.5 mm, and dispersed for 12 hours. Then, the slurry was added with 4 g of benzothiazolinone sodium salt and water so that the concentration of Nucleating agent Y could become 10 weight % to obtain microparticle dispersion of the nucleating agent. The particles of Nucleating agent Y contained in the dispersion obtained as described above had a median diameter of 0.34  $\mu\text{m}$ , maximum particle diameter of 3.0  $\mu\text{m}$  or less, and variation coefficient of 19% for the particle diameter. The obtained dispersion was filtered through a polypropylene filter having a pore size of 3.0  $\mu\text{m}$  to remove dusts and so forth, and stored.

Preparation of Solid Microparticle Dispersion of  
Development Accelerator W

5 In an amount of 10 kg of Development accelerator W, 10 kg of 20 weight % aqueous solution of denatured polyvinyl alcohol (Poval MP203, produced by Kuraray Co., Ltd.) and 20 kg of water were mixed sufficiently to form slurry. The 10 slurry was fed by a diaphragm pump to a sand mill of horizontal type (UVM-2, produced by Imex Co.) containing zirconia beads having a mean diameter of 0.5 mm, and dispersed for 5 hours. Then, the slurry was added with water so that the concentration of Development accelerator W 15 could become 20 weight % to obtain a microparticle dispersion of Development accelerator W. The particles of Development accelerator W contained in the dispersion obtained as described above had a median diameter of 0.5  $\mu\text{m}$ , maximum particle diameter of 2.0  $\mu\text{m}$  or less, and variation coefficient of 18% for the mean particle diameter. The obtained dispersion was filtered through a polypropylene filter having a pore size of 3.0  $\mu\text{m}$  to remove dusts and so forth, and stored.

Preparation of Coating Solution for Image-forming  
Layer

Silver behenate dispersion A prepared above was added with the following binder, components and Silver halide emulsion A in the indicated amounts per mole of silver in 35 Silver behenate dispersion A, and added with water to prepare a coating solution for image-forming layer. After the completion, the solution was degassed under reduced pressure of 0.54 atm for 45 minutes. The coating solution showed pH of 7.3–7.7 and viscosity of 40–50  $\text{mpa}\cdot\text{s}$  at 25° C.

|    |                                                                                                                                |                                                                                 |
|----|--------------------------------------------------------------------------------------------------------------------------------|---------------------------------------------------------------------------------|
| 45 | Binder: LACSTAR 3307B<br>(SBR latex, produced by Dai-Nippon<br>Ink & Chemicals, Inc., glass<br>transition temperature: 17° C.) | 397 g as solid                                                                  |
| 50 | 1,1-Bis(2-hydroxy-3,5-dimethyl-<br>phenyl)-3,5,5-trimethylhexane                                                               | 149 g as solid                                                                  |
| 55 | Organic polyhalogenated compound A                                                                                             | 43.6 g as solid                                                                 |
|    | Organic polyhalogenated compound B                                                                                             | 3.8 g as solid                                                                  |
| 60 | Organic polyhalogenated compound C                                                                                             | 2.25 g as solid                                                                 |
|    | Sodium ethylthiosulfonate                                                                                                      | 0.47 g                                                                          |
|    | Benzotriazole                                                                                                                  | 1.02 g                                                                          |
|    | Polyvinyl alcohol (PVA-235, produced<br>by Kuraray Co., Ltd.)                                                                  | 10.8 g                                                                          |
| 65 | 6-Isopropylphthalazine                                                                                                         | 17.0 g                                                                          |
|    | Compound Z                                                                                                                     | 9.7 g as solid                                                                  |
|    | Nucleating agent Y                                                                                                             | 15.3 g as solid                                                                 |
|    | Dye A<br>(added as a mixture with low<br>molecular weight gelatin having<br>mean molecular weight of 15000)                    | Amount giving optical<br>density of 0.3 at 783 nm<br>(about 0.37 g as solid)    |
|    | Silver halide emulsion A                                                                                                       | 0.06 mole as Ag                                                                 |
|    | Compound A as preservative                                                                                                     | 40 ppm in the coating solution<br>(2.5 $\text{mg}/\text{m}^2$ as coated amount) |
|    | Methanol                                                                                                                       | 2 weight % as to total solvent<br>amount in the coating solution                |
|    | Ethanol                                                                                                                        | 1 weight % as to total solvent<br>amount in the coating solution                |

37

(The coated film showed a glass transition temperature of 17° C.)



#### Preparation of Coating Solution for Lower Protective Layer

In an amount of 943 g of a polymer latex solution containing copolymer of methyl methacrylate/styrene/2-ethylhexyl acrylate/2-hydroxyethyl methacrylate/acrylic acid=58.9/8.6/25.4/5.1/2 (weight %) (glass transition temperature as copolymer: 46° C. (calculated value), solid content: 21.5 weight %, containing 100 ppm of Compound A and further containing Compound D as a film-forming aid in an amount of 15 weight % relative to solid content of the latex so that the glass transition temperature of the coating solution could become 24° C., mean particle diameter: 116 nm) was added with water, 1.62 g of Compound E, 112.7 g of aqueous solution of Organic polyhalogenated compound C, 11.54 g as solid content of Development accelerator W, 1.58 g of matting agent (polystyrene particles, mean particle diameter: 7  $\mu$ m, variation coefficient of 8% for mean particle diameter) and 29.4 g of polyvinyl alcohol (PVA-235, Kuraray Co., Ltd.) and further added with water to form a coating solution (containing 2 weight % of methanol solvent).

38

After the completion, the solution was degassed under reduced pressure of 0.47 atm for 60 minutes. The coating solution showed pH of 5.4, and viscosity of 39 mPa·s at 25° C.

5 Preparation of Coating Solution for Upper Protective Layer

In an amount of 649 g of a polymer latex solution containing copolymer of methyl methacrylate/styrene/2-ethylhexyl acrylate/2-hydroxyethyl methacrylate/acrylic acid=58.9/8.6/25.4/5.1/2 (weight %) (glass transition temperature as copolymer: 46° C. (calculated value), solid content: 21.5 weight %, containing 100 ppm of Compound A and further containing Compound D as a film-forming aid in an amount of 15 weight % relative to solid content of the latex so that the glass transition temperature of the coating solution could become 24° C., mean particle diameter: 72 nm) was added with water, 6.30 g of 30 weight % solution of carnauba wax (Cellosol 524, silicone content: less than 5 ppm, Chukyo Yushi Co., Ltd.), 0.23 g of Compound C, 0.93 g of Compound E, 7.95 g of Compound F, 1.8 g of Compound H, 1.18 g of matting agent (polystyrene particles, mean particle diameter: 7  $\mu$ m, variation coefficient of 8% for mean particle diameter) and 12.1 g of polyvinyl alcohol (PVA-235, Kuraray Co., Ltd.), and further added with water to form a coating solution (containing 1.5 weight % of methanol solvent) After the completion, the solution was degassed under reduced pressure of 0.47 atm for 60 minutes. The coating solution showed pH of 2.8, and viscosity of 30 mPa·s at 25° C.



#### Preparation of PET Support with Back Layer and Undercoat Layer

65 (1) Preparation of PET Support  
Polyethylene terephthalate having IV (intrinsic viscosity) of 0.66 (measured in phenol/tetrachloroethane=6/4 (weight

ratio) at 25° C.) was obtained by using terephthalic acid and ethylene glycol in a conventional manner. The product was pelletized, dried at 130° C. for 4 hours, melted at 300° C., then extruded from a T-die and rapidly cooled to form an unstretched film having a thickness of 120  $\mu\text{m}$  after thermal fixation.

The film was stretched along the longitudinal direction by 3.3 times using rollers of different peripheral speeds, and then stretched along the transverse direction by 4.5 times using a tenter. The temperatures used for these operations were 110° C. and 130° C., respectively. Then, the film was subjected to thermal fixation at 240° C. for 20 seconds, and relaxed by 4% along the transverse direction at the same temperature. Then, the chuck of the tenter was released, the both edges of the film were knurled, and the film was rolled up at 4.8 kg/cm<sup>2</sup>. Thus, a roll of a film having a width of 2.4 m, length of 3500 m, and thickness of 120  $\mu\text{m}$  was obtained.

(2) Preparation of undercoat layers and back layers  
(i) First undercoat layer

The aforementioned PET support was subjected to a corona discharge treatment of 0.375 kV·A·minute/m<sup>2</sup>, then coated with a coating solution having the following composition in an amount of 6.2 ml/m<sup>2</sup>, and dried at 125° C. for 30 seconds, 150° C. for 30 seconds, and 185° C. for 30 seconds.

|                                                                                                                                        |                                      |  |
|----------------------------------------------------------------------------------------------------------------------------------------|--------------------------------------|--|
| Latex A                                                                                                                                | 280 g                                |  |
| KOH                                                                                                                                    | 0.5 g                                |  |
| Polystyrene microparticles<br>(mean particle diameter; 2 $\mu\text{m}$ ,<br>variation coefficient of 7% for<br>mean particle diameter) | 0.03 g                               |  |
| 2,4-Dichloro-6-hydroxy-s-triazine                                                                                                      | 1.8 g                                |  |
| Compound Bc-C                                                                                                                          | 0.097 g                              |  |
| Distilled water                                                                                                                        | Amount giving total weight of 1000 g |  |

(ii) Second undercoat layer

A coating solution having the following composition was coated on the first undercoat layer in an amount of 5.5 ml/m<sup>2</sup> and dried at 125° C. for 30 seconds, 150° C. for 30 seconds, and 170° C. for 30 seconds.

|                                                                                    |                                         |  |
|------------------------------------------------------------------------------------|-----------------------------------------|--|
| Deionized gelatin<br>(Ca <sup>2+</sup> content; 0.6 ppm,<br>jelly strength; 230 g) | 10.0 g                                  |  |
| Acetic acid (20% aqueous solution)                                                 | 10.0 g                                  |  |
| Compound Bc-A                                                                      | 0.04 g                                  |  |
| Methylcellulose (2% aqueous solution)                                              | 25.0 g                                  |  |
| Emalex 710 (produced by Nihon<br>Emulsion Co.)                                     | 0.3 g                                   |  |
| Distilled water                                                                    | Amount giving total<br>weight of 1000 g |  |

(iii) First back layer

The surface of the support opposite to the surface coated with the undercoat layers was subjected to a corona discharge treatment of 0.375 kV·A·minute/m<sup>2</sup>, coated with a coating solution having the following composition in an amount of 13.8 ml/m<sup>2</sup>, and dried at 125° C. for 30 seconds, 150° C. for 30 seconds, and 185° C. for 30 seconds.

|                                                                       |        |  |
|-----------------------------------------------------------------------|--------|--|
| Julimer ET-410<br>(30% aqueous dispersion<br>Nihon Junyaku Co., Ltd.) | 23.0 g |  |
|-----------------------------------------------------------------------|--------|--|

-continued

|                                                                                                                                 |                                                                     |
|---------------------------------------------------------------------------------------------------------------------------------|---------------------------------------------------------------------|
| Alkali-treated gelatin<br>(molecular weight; about 10000,<br>Ca <sup>2+</sup> content; 30 ppm)                                  | 4.44 g                                                              |
| Deionized gelatin<br>(Ca <sup>2+</sup> content; 0.6 ppm)                                                                        | 0.84 g                                                              |
| Compound Bc-A                                                                                                                   | 0.02 g                                                              |
| Dye Bc-A                                                                                                                        | Amount giving optical density of<br>1.3-1.4 at 783 nm, about 0.88 g |
| 10 Polyoxethylene phenyl ether                                                                                                  | 1.7 g                                                               |
| Sumitex Resin M-3<br>(8% aqueous solution,<br>water-soluble melamine compound,<br>Sumitomo Chemical Co., Ltd.)                  | 15.0 g                                                              |
| 15 FS-10D (aqueous dispersion of<br>Sb-doped Sb <sub>2</sub> O <sub>3</sub> acicular grains,<br>Ishihara Sangyo Kaisha, Ltd.)   | 24.0 g                                                              |
| Polystyrene microparticles<br>(mean diameter; 2.0 $\mu\text{m}$ ,<br>variation coefficient of 7%<br>for mean particle diameter) | 0.03 g                                                              |
| Distilled water                                                                                                                 | Amount giving total<br>weight of 1000 g                             |

25 (iv) Second back layer

A coating solution having the following composition was coated on the first back layer in an amount of 5.5 ml/m<sup>2</sup> and dried at 125° C. for 30 seconds, 150° C. for 30 seconds, and 170° C. for 30 seconds.

|                                                                                                             |                                         |
|-------------------------------------------------------------------------------------------------------------|-----------------------------------------|
| 30 Julimer ET-410<br>(30% aqueous dispersion Nihon Junyaku Co., Ltd.)                                       | 57.5 g                                  |
| 35 Polyoxethylene phenyl ether                                                                              | 1.7 g                                   |
| Sumitex Resin M-3<br>(8% aqueous solution, water-soluble melamine<br>compound, Sumitomo Chemical Co., Ltd.) | 15.0 g                                  |
| Cellosol 524<br>(30% aqueous solution, Chukyo Yushi Co., Ltd.)                                              | 6.6 g                                   |
| Distilled water                                                                                             | Amount giving total<br>weight of 1000 g |

50 (v) Third back layer

The same coating solution as the first undercoat layer was coated on the second back layer in an amount of 6.2 ml/m<sup>2</sup> and dried at 125° C. for 30 seconds, 150° C. for 30 seconds, and 185° C. for 30 seconds.

55 (vi) Fourth back layer

A coating solution having the following composition was coated on the third back layer in an amount of 13.8 ml/m<sup>2</sup> and dried at 125° C. for 30 seconds, 150° C. for 30 seconds, and 170° C. for 30 seconds.

|                                                                                                                                                                 |                                         |
|-----------------------------------------------------------------------------------------------------------------------------------------------------------------|-----------------------------------------|
| 55 Latex B                                                                                                                                                      | 286 g                                   |
| Compound Bc-B                                                                                                                                                   | 2.7 g                                   |
| Compound Bc-C                                                                                                                                                   | 0.6 g                                   |
| Compound Bc-D                                                                                                                                                   | 0.5 g                                   |
| 2,4-Dichloro-6-hydroxy-s-triazine                                                                                                                               | 2.5 g                                   |
| Poly(methyl methacrylate)<br>(10% aqueous dispersion, mean particle<br>diameter: 5.0 $\mu\text{m}$ , variation coefficient of 7% for<br>mean particle diameter) | 7.7 g                                   |
| Distilled water                                                                                                                                                 | Amount giving total<br>weight of 1000 g |



## Latex A

Core/shell type latex comprising 90 weight % of core and 10 weight % of shell, core: vinylidene chloride/methyl acrylate/methyl methacrylate/acrylonitrile/acrylic acid=93/3/3/0.9/0.1 (weight %), shell: vinylidene chloride/methyl acrylate/methyl methacrylate/acrylonitrile/acrylic acid=88/3/3/3/3 (weight %), weight average molecular weight; 38000)

## Latex B

Latex of copolymer of methyl methacrylate/styrene/2-ethylhexyl acrylate/2-hydroxyethyl methacrylate/acrylic acid=59/9/26/5/1 (weight %)

(3) Heat treatment during transportation

(3-1) Heat treatment

The PET support with back layers and undercoat layers prepared as described above was introduced into a heat treatment zone having a total length of 200 m set at 160° C., and transported at a tension of 2 kg/cm<sup>2</sup> and a transportation speed of 20 m/minute.

(3-2) Post-heat treatment

Following the aforementioned heat treatment, the support was subjected to a post-heat treatment by passing it through a zone at 40° C. for 15 seconds, and rolled up. The rolling up tension for this operation was 10 kg/cm<sup>2</sup>.

## Preparation of Photothermographic Materials

On the undercoat layers of the aforementioned PET support on the side coated with the first and second undercoat layers, the aforementioned coating solution for image-forming layer was coated so that the coated silver amount could be 1.5 g/m<sup>2</sup> by the slide bead method disclosed in JP-A-2000-2964, FIG. 1. Further, the aforementioned coating solution for lower protective layer was coated on the image-forming layer simultaneously with the coating solution for image-forming layer as stacked layers, so that the coated solid content of the polymer latex could be 1.31 g/m<sup>2</sup>. Then, the aforementioned coating solution for upper protective layer was coated on the coated layers, so that the

coated solid content of the polymer latex could be 3.11 g/m<sup>2</sup> to obtain a photothermographic material.

After the coating, the layers were dried in a horizontal drying zone (the support was at an angle of 1.5–3° to the horizontal direction of the coating machine) under the following conditions: dry-bulb temperature of 70–75° C., dew point of 8–25° C. and liquid film surface temperature of 35–60° C. for both of the constant rate drying process and the decreasing rate drying process. The saturation swelling time in distilled water at 21° C. was varied as shown in Table 1 by changing the liquid film surface temperature. After the drying, the material was rolled up under the conditions of a temperature of 25±5° C. and relative humidity of 45±10%, and the material was rolled up in such a rolled shape that the image-forming layer should be exposed to the outside so as to conform to the subsequent processing (image-forming layer outside roll). The humidity in the package of the photosensitive material was 20–40% of relative humidity (measured at 25° C.). Each of the obtained photothermographic material showed a film surface pH of 5.0 and Beck's smoothness of 850 seconds for the image-forming layer side. The opposite surface showed a film surface pH of 5.9 and Beck's smoothness of 560 seconds.

## Evaluation of Photographic Performance

## (Light Exposure)

The obtained photothermographic material was light exposed for  $1.2 \times 10^{-8}$  second at a mirror revolution number of 60000 rpm by using a laser light-exposure apparatus of single channel cylindrical internal surface scanning type provided with a semiconductor laser with a beam diameter (½ of FWHM of beam intensity) of 12.56  $\mu\text{m}$ , laser output of 50 mW and output wavelength of 783 nm. The overlap coefficient of the light exposure was 0.449, and the laser energy density on the photothermographic material surface was 75  $\mu\text{J}/\text{cm}^2$ .

## (Heat Development)

Each light-exposed photothermographic material was heat-developed by using such a heat development apparatus as shown in FIG. 1. The roller surface material of the heat development section was composed of silicone rubber, and the flat surface consisted of Teflon non-woven fabric. The heat development was performed at a transportation line speed of 150 cm/minute. The heat development treatment was performed in the preheating section for 12.2 seconds (Driving units of the preheating section and the heat development section were independent from each other, and speed difference as to the heat development section was adjusted to –0.5% to –1%). Temperatures of the metallic rollers and processing times for each preheating part are as follows: first roller, 67° C. for 2.0 seconds; second roller, 82° C. for 2.0 seconds; third roller, 98° C. for 2.0 seconds; fourth roller, 107° C. for 2.0 seconds; fifth roller, 115° C. for 2.0 seconds; and sixth roller, 120° C. for 2.0 seconds), in the heat development section at 120° C. (surface temperature of photothermographic material) for 17.2 seconds, and in the gradual cooling section for 13.6 seconds. The temperature precision as for the transverse direction was ±0.5° C. As for

each roller temperature setting, the temperature precision was secured by using a length of rollers longer than the width of the photothermographic material (for example, width of 61 cm) by 5 cm for the both sides and also heating the protruding portions. Since the rollers showed marked temperature decrease at the both end portions, the temperature of the portions protruding by 5 cm from the end of the photothermographic material was controlled to be higher than that of the roller center by 1–3° C., so that uniform image density of a finished developed image could be obtained for the whole photothermographic material surface (for example, within a width of 61 cm).

#### Evaluation of Photographic Performance

Development humidity dependency was evaluated as a difference of line width obtained for a photothermographic material that was left in an environment of 25° C. and relative humidity of 80% for 16 hours, exposed for a line width of 60  $\mu\text{m}$  in that environment and subjected to the heat development, and a photothermographic material that was left in an environment of 25° C. and relative humidity of 10% for 16 hours, exposed with the same condition as above in that environment and subjected to the heat development. Further, Dmin (fog) and Dmax (maximum density) were also evaluated in each of the environments. The measurement of density was performed by using Macbeth TD904 densitometer (visible density).

#### Measurement of Saturation Swelling Time

Each photothermographic material was conditioned for its moisture content at 30° C. and relative humidity of 40% for 1 day. A given amount of distilled water at 21° C. was dropped on the image-forming layer side of the photothermographic material, and time required until swelling reached plateau was measured to obtain saturation swelling time.

The results of the above evaluations for each photothermographic material are shown in Table 1.

times were 60 seconds or more showed low development humidity dependency for the line width and they could secure sufficient image density (Dmax) even in such a low humidity environment of 25° C. and relative humidity of 10%.

Further, since Samples 9 and 10 of the photothermographic materials not utilizing a nucleating agent did not show the development humidity dependency, it can be seen that the development humidity dependency is a phenomenon characteristic of photothermographic materials containing a nucleating agent. Moreover, it can be seen that it is more effective to use a substituted alkene derivative such as Nucleating agent Y rather than hydrazine as the nucleating agent.

The above results clearly demonstrated the advantages of the present invention.

#### Example 2

##### Preparation of Photothermographic Materials

The coating solution for image-forming layer and the coating solution for lower protective layer of Example 1 were simultaneously coated as stacked layers in the same manner as in Example 1. Then, the coating solution for upper protective layer shown in Example 1 was coated to prepare photothermographic materials, provided that coated latex solid content was changed as shown in Table 2 and coated amounts of the components other than the latex were adjusted so that they could be the same as the coated amount of latex solid content in Example 1, 3.11 g/m<sup>2</sup>. Evaluations of photographic properties were performed in the exactly same manner as in Example 1.

The results of the above evaluations for each photothermographic material are shown in Table 2.

TABLE 1

| Photothermographic material | Liquid film surface temperature (° C.) | Saturation swelling time (second) | Under environment of 25° C. and 80% RH |      | Under environment of 25° C. and 10% RH |      | Variation of line width ( $\mu\text{m}$ ) |
|-----------------------------|----------------------------------------|-----------------------------------|----------------------------------------|------|----------------------------------------|------|-------------------------------------------|
|                             |                                        |                                   | Dmin                                   | Dmax | Dmin                                   | Dmax |                                           |
| 1                           | 35                                     | 35                                | 0.13                                   | 4.0  | 0.12                                   | 2.8  | 15                                        |
| 2                           | 38                                     | 47                                | 0.13                                   | 4.0  | 0.12                                   | 3.2  | 13                                        |
| 3                           | 40                                     | 56                                | 0.13                                   | 4.0  | 0.12                                   | 3.6  | 13                                        |
| 4 (Invention)               | 43                                     | 65                                | 0.12                                   | 4.0  | 0.12                                   | 3.9  | 9                                         |
| 5 (Invention)               | 45                                     | 72                                | 0.12                                   | 4.1  | 0.12                                   | 4.0  | 7                                         |
| 6 (Invention)               | 50                                     | 80                                | 0.12                                   | 4.1  | 0.12                                   | 4.1  | 5                                         |
| 7 (Invention)               | 55                                     | 89                                | 0.12                                   | 4.1  | 0.12                                   | 4.1  | 4                                         |
| 8 (Invention)               | 60                                     | 96                                | 0.12                                   | 4.1  | 0.12                                   | 4.1  | 4                                         |
| 9                           | 35                                     | 35                                | 0.12                                   | 1.6  | 0.12                                   | 1.6  | 0                                         |
| 10                          | 50                                     | 80                                | 0.12                                   | 1.6  | 0.12                                   | 1.6  | 0                                         |
| 11                          | 35                                     | 35                                | 0.14                                   | 3.8  | 0.13                                   | 2.2  | 20                                        |
| 12 (Invention)              | 50                                     | 80                                | 0.13                                   | 3.8  | 0.12                                   | 3.6  | 8                                         |

In Photothermographic materials 9 and 10, image-forming layers did not contain Nucleating agent Y.

In Photothermographic materials 11 and 12, image-forming layers contained N-(2-methoxyphenyl)-N'-formylhydrazine instead of Nucleating agent Y in the same molar amounts.

From the results shown in Table 1, it can be seen that the photothermographic materials of which saturation swelling

TABLE 2

| Photothermographic material | layer | Coated amount of latex in upper protective layers (μm) | Total thickness of protective layers (μm) | Liquid film surface temperature (° C.) | Saturation swelling time (second) | Under environment of 25° C. and 80% RH |      | Under environment of 25° C. and 10% RH |      | Variation of line width (μm) |
|-----------------------------|-------|--------------------------------------------------------|-------------------------------------------|----------------------------------------|-----------------------------------|----------------------------------------|------|----------------------------------------|------|------------------------------|
|                             |       |                                                        |                                           |                                        |                                   | Dmin                                   | Dmax | Dmin                                   | Dmax |                              |
| 2                           |       | 3.11 g/m <sup>2</sup>                                  | 4.2                                       | 38                                     | 47                                | 0.13                                   | 4.0  | 0.12                                   | 3.2  | 13                           |
| 6 (Invention)               |       | 3.11 g/m <sup>2</sup>                                  | 4.2                                       | 50                                     | 80                                | 0.12                                   | 4.1  | 0.12                                   | 4.1  | 5                            |
| 13 (Invention)              |       | 2.33 g/m <sup>2</sup>                                  | 3.5                                       | 50                                     | 75                                | 0.12                                   | 4.1  | 0.12                                   | 4.0  | 6                            |
| 14 (Invention)              |       | 1.56 g/m <sup>2</sup>                                  | 2.7                                       | 50                                     | 68                                | 0.12                                   | 4.0  | 0.12                                   | 4.0  | 7                            |
| 15 (Invention)              |       | 1.28 g/m <sup>2</sup>                                  | 2.5                                       | 50                                     | 63                                | 0.12                                   | 4.0  | 0.12                                   | 3.9  | 9                            |

From the results shown in Table 2, it can be seen that the photothermographic materials of which saturation swelling times were 60 seconds or more showed low development humidity dependency for the line width and they could secure sufficient image density (Dmax) even in such a low humidity environment of 25° C. and relative humidity of 10%. In particular, it can be seen that the photothermographic materials having a protective layer thickness of 3 μm or more showed better performance.

The above results clearly demonstrated the advantages of the present invention.

### Example 3

#### Preparation of Photothermographic Material

The coating solution for image-forming layer and the coating solution for lower protective layer shown in Example 1 were simultaneously coated as stacked layers in the same manner as in Example 1. Then, the following coating solutions for two kinds of protective layers, the coating solution for intermediate protective layer and the coating solution for uppermost protective layer, were simultaneously coated as stacked layers so that the coated amount of polymer latex solid content in the intermediate protective layer could be 1.97 g/m<sup>2</sup> and the coated amount of polymer latex solid content in the uppermost protective layer should be 1.07 g/m<sup>2</sup> to prepare a photothermographic material.

#### Preparation of Coating Solution for Intermediate Protective Layer

In an amount of 625 g of polymer latex solution containing copolymer of methyl methacrylate/styrene/2-ethylhexyl acrylate/2-hydroxyethyl methacrylate/acrylic acid=58.9/8.6/25.4/5.1/2 (weight %) (glass transition temperature of the copolymer: 46° C. (calculated value), solid content: 21.5 wt %, containing Compound A at a concentration of 100 ppm and further containing Compound D as a film-forming aid in an amount of 15 wt % relative to solid content of the latex so that the glass transition temperature of coating solution could become 24° C., mean particle diameter: 72 nm) was added with H<sub>2</sub>O, 0.23 g of Compound C, 0.13 g of Compound E, 12.1 g of Compound F, 2.75 g of Compound H and 11.5 g of polyvinyl alcohol (PVA-235, Kuraray Co., Ltd.) and further added with H<sub>2</sub>O to form a coating solution (containing 0.5 weight % of methanol solvent). After the completion, the coating solution was degassed at a pressure of 0.47 atm for 60 minutes. The coating solution showed pH of 2.6 and viscosity of 50 mpa·s at 25° C.

#### Preparation of Coating Solution for Uppermost Protective Layer

In an amount of 649 g of polymer latex solution containing copolymer of methyl methacrylate/styrene/2-ethylhexyl

acrylate/2-hydroxyethyl methacrylate/acrylic acid=58.9/8.6/25.4/5.1/2 (weight %) (glass transition temperature of the copolymer: 46° C. (calculated value), solid content: 21.5 weight %, containing Compound A at a concentration of 100 ppm and further containing Compound D as a film-forming aid in an amount of 15 weight % relative to solid content of the latex so that the glass transition temperature of coating solution could become 24° C., mean particle diameter: 116 nm) was added with H<sub>2</sub>O, 0.23 g of Compound C, 1.85 g of Compound E, 1.0 g of Compound G, 18.4 g of 30 weight % solution of carnauba wax (Cellosol 524, Chukyo Yushi Co., Ltd., silicone content: less than 5 ppm), 3.45 g of matting agent (polystyrene particles, mean diameter: 7 μm, variation coefficient for mean particle diameter: 8%, 3.45 g) and 26.5 g of polyvinyl alcohol (PVA-235, Kuraray Co., Ltd., 26.5 g) and further added with H<sub>2</sub>O to form a coating solution (containing 3 weight % of methanol solvent).

After the completion, the coating solution was degassed at a pressure of 0.47 atm for 60 minutes. The coating solution showed pH of 5.2 and viscosity of 24 mpa·s at 25° C.

The obtained photothermographic materials were evaluated in the same manner as in Example 1. As a result, the results of Example 1 were substantially reproduced. That is, the photothermographic material of which saturation swelling time was 60 seconds or more showed low development humidity dependency for the line width and it could secure sufficient image density (Dmax) even in such a low humidity environment of 25° C. and relative humidity of 10%. Therefore, the advantages of the present invention were clearly demonstrated.

### Example 4

The same samples as used in Example 1 were exposed by using a cylinder external surface scanning type multichannel exposure apparatus (provided with 30 of 50 mW semiconductor laser heads, laser energy density on the photothermographic material surface: 75 μJ/cm<sup>2</sup>), and subjected to heat development in the same manner as in Example 1. As a result, the photothermographic materials of the present invention showed low development humidity dependency for the line width and they could secure sufficient image density (Dmax) even in such a low humidity environment of 25° C. and relative humidity of 10%. Therefore, the advantages of the present invention were clearly demonstrated.

What is claimed is:

1. A photothermographic material having an image-forming layer that contains at least a non-photosensitive silver salt of an organic acid, a photosensitive silver halide, a nucleating agent and a binder on a support, and a protective layer at a position remote from the support compared with the image-forming layer, which shows a saturation swelling time of 60 seconds to 5 minutes in distilled water at 21° C.

2. The photothermographic material according to claim 1, wherein the saturation swelling time is 80 seconds or longer.
3. The photothermographic material according to claim 1, wherein the binder of the image-forming layer comprises 50 weight % or more of latex of a polymer showing a glass transition temperature of -30° C. to 40° C.
4. The photothermographic material according to claim 1, wherein the protective layer has a thickness of 3  $\mu$ m or more.
5. A method for forming images, which comprises exposing imagewise the photothermographic material of claim 1 to light; and subjecting the photothermographic material to a heat treatment at a line speed of 140 cm/minute or higher to form said images.
6. A method for forming images, which comprises exposing the photothermographic material according to claim 1 for an exposure time of 10<sup>-7</sup> second or less.
7. A method for forming images, which comprises exposing the photothermographic material according to claim 1 by using a multi-channel light source having two or more of laser heads.
8. A method for forming images, which comprises exposing imagewise the photothermographic material of claim 1 to light; heating the photothermographic material at a temperature of 80° C. or higher but lower than 115° C. for 5 seconds or more so as not to develop images; and heat-developing the photothermographic material at a temperature of 110–140° C. to form said images.
9. The photothermographic material of claim 1, wherein said non-photosensitive silver salt of an organic acid is a silver salt of a long chained aliphatic carboxylic acid having 10 to 30 carbon atoms.
10. The photothermographic material of claim 1, wherein said non-photosensitive silver salt of an organic acid is selected from the group consisting of silver behenate, silver arachidinate, silver stearate, silver oleate, silver laurate, silver caproate, silver myristate, silver palmitate, silver maleate, silver fumarate, silver tartrate, silver linoleate, silver butyrate, silver camphorate, and mixtures thereof.
11. The photothermographic material of claim 1, wherein said non-photosensitive silver salt of an organic acid is used in amount of 0.1 to 5 g/m<sup>2</sup>.
12. The photothermographic material of claim 1, wherein said photosensitive silver halide is selected from the group consisting of silver chloride, silver chlorobromide, silver bromide, silver iodobromide and silver chloroiodobromide.
13. The photothermographic material of claim 1, wherein said nucleating agent is in the amount of 1×10<sup>-6</sup> mole to one mole of silver.
14. The photothermographic material of claim 1, wherein an acid formed by hydration of a diphosphorus pentoxide or a salt thereof is used with said nucleating agent.
15. The photothermographic material of claim 1, further comprising a compound selected from the group consisting

- of a benzoic acid compound, a mercury salt, an organic halide, a mercapto compound, a disulfide compound and a thione compound.
16. The photothermographic material of claim 1, wherein said binder of the protective layer comprises a polymer latex having a glass transition temperature of 25° C. to 70° C.
17. The photothermographic material of claim 1, further comprising a back layer, wherein the binder in said back layer comprises a polymer latex having a glass transition temperature of 25° C. to 70° C.
18. The photothermographic material of claim 1, wherein the binder of the protective layer further comprises a polymer latex, wherein said polymer latex shows a minimum filming forming temperature of -30° C. to 90° C.
19. The photothermographic material of claim 1, wherein the binder of the protective layer further comprises a polymer latex, wherein said polymer latex is selected from the group consisting of acrylic resins, polyvinyl acetate resins, polyester resins, polyurethane resins, rubber resins, polyolefin resins, and copolymers of monomers of the resins thereof.
20. The photothermographic material of claim 3, wherein said polymer latex in said image-forming layer is selected from the group consisting of latex of methyl methacrylate/ethyl acrylate/methacrylic acid copolymer, latex of methyl methacrylate/butadiene/itaconic acid polymer, latex of ethyl acrylate/methacrylic acid copolymer, latex of methyl methacrylate/2-ethylhexyl acrylate/styrene/acrylic acid copolymer, latex of styrene/butadiene/acrylic acid copolymer, latex of styrene/butadiene/divinylbenzene/methacrylic acid copolymer, latex of methyl methacrylate/vinyl chloride/acrylic acid copolymer, and latex of vinylidene chloride/ethyl acrylate/acrylonitrile/methacrylic acid copolymer.
21. The photothermographic material of claim 3, wherein said binder of the protective layer comprises a polymer latex having a glass transition temperature of 25° C. to 70° C.
22. The photothermographic material of claim 3, further comprising a back layer, wherein the binder of said back layer comprises a polymer latex having a glass transition temperature of 25° C. to 70° C.
23. The photothermographic material of claim 3, 21 or 22, wherein said polymer latex of any of said layers shows a minimum filming forming temperature of -30° C. to 90° C.
24. The photothermographic material of claim 16 or 17, wherein said polymer latex of any of said layers shows a minimum filming forming temperature of -30° C. to 90° C.
25. The photothermographic material of claim 16 or 17, wherein said polymer latex of any of said layers is selected from the group consisting of acrylic resins, polyvinyl acetate resins, polyester resins, polyurethane resins, rubber resins, polyolefin resins, and copolymers of monomers of the resins thereof.

\* \* \* \* \*